



US008293439B2

(12) **United States Patent**  
**Fujiwara et al.**

(10) **Patent No.:** **US 8,293,439 B2**  
(45) **Date of Patent:** **Oct. 23, 2012**

(54) **ELECTROPHOTOGRAPHIC PHOTORECTOR, METHOD OF MANUFACTURING ELECTROPHOTOGRAPHIC PHOTORECTOR, IMAGE FORMING APPARATUS, AND PROCESS CARTRIDGE**

(75) Inventors: **Yukio Fujiwara**, Numazu (JP); **Hidetoshi Kami**, Numazu (JP); **Kazuhiko Egawa**, Numazu (JP); **Shinji Nohsho**, Numazu (JP); **Mayumi Yoshihara**, Numazu (JP); **Mioko Matsumoto**, Susono (JP); **Kohsuke Yamamoto**, Zama (JP)

(73) Assignee: **Ricoh Company, Ltd.**, Tokyo (JP)

(\*) Notice: Subject to any disclaimer, the term of this patent is extended or adjusted under 35 U.S.C. 154(b) by 224 days.

(21) Appl. No.: **12/723,058**

(22) Filed: **Mar. 12, 2010**

(65) **Prior Publication Data**

US 2010/0232831 A1 Sep. 16, 2010

(30) **Foreign Application Priority Data**

Mar. 13, 2009 (JP) ..... 2009-061268  
Mar. 3, 2010 (JP) ..... 2010-046096

(51) **Int. Cl.**  
**G03G 5/147** (2006.01)

(52) **U.S. Cl.** ..... **430/66; 430/56; 430/58.2; 430/58.7;**  
399/159

(58) **Field of Classification Search** ..... 430/56,  
430/58.2, 58.7, 66; 399/159

See application file for complete search history.

(56) **References Cited**

U.S. PATENT DOCUMENTS

6,861,188 B2 3/2005 Ikegami et al.  
(Continued)

FOREIGN PATENT DOCUMENTS

JP 57-78402 5/1982  
(Continued)

OTHER PUBLICATIONS

“Blade cleaning system for polymerized and small size toner”,  
Hyakutake et al., Japan Hardcopy Fall Meeting, 2001, pp. 24-27.

(Continued)

Primary Examiner — Peter Vajda

(74) Attorney, Agent, or Firm — Cooper & Dunham LLP

(57) **ABSTRACT**

An electrophotographic photoreceptor including a conductive substrate, a photosensitive layer, and a surface layer, which satisfies the following inequations:

$0.005 < WRa(LMH) < 0.03$  (i)

$0.010 < WRa(LHH) < 0.03$  (ii)

$0.005 < WRa(LML) < 0.20$  (iii)

$WRa(LLH) > WRa(LMH)$  (iv)

$WRa(LLH) > WRa(LHH)$  (v)

wherein WRa ( $\mu m$ ) represents a center-line average roughness of frequency components LHH, LHL, LMH, LML, LLH, and LLL that are obtained by subjecting a one-dimensional data array of a surface profile of the electrophotographic photoreceptor to wavelet transformation multiresolution analysis so as to be separated into 6 frequency components; thinning a one-dimensional data array of the lowest frequency component so that the number of data array is reduced to 1/40; and subjecting the thinned one-dimensional data array to wavelet transformation multiresolution analysis so as to be separated into the 6 frequency components LHH, LHL, LMH, LML, LLH, and LLL.

**12 Claims, 24 Drawing Sheets**



## U.S. PATENT DOCUMENTS

|              |    |         |                 |    |             |         |
|--------------|----|---------|-----------------|----|-------------|---------|
| 6,936,388    | B2 | 8/2005  | Suzuki et al.   | JP | 2002-341572 | 11/2002 |
| 7,018,755    | B2 | 3/2006  | Ikegami et al.  | JP | 2003-131537 | 5/2003  |
| 7,160,658    | B2 | 1/2007  | Suzuki et al.   | JP | 2003-241408 | 8/2003  |
| 7,177,570    | B2 | 2/2007  | Nagame et al.   | JP | 2003-270840 | 9/2003  |
| 7,267,916    | B2 | 9/2007  | Sugino et al.   | JP | 2004-54001  | 2/2004  |
| 7,314,693    | B2 | 1/2008  | Ikegami et al.  | JP | 2004-61359  | 2/2004  |
| 7,381,511    | B2 | 6/2008  | Ikegami et al.  | JP | 2004-258588 | 9/2004  |
| 2007/0031746 | A1 | 2/2007  | Toshine et al.  | JP | 2006-53576  | 2/2006  |
| 2007/0196749 | A1 | 8/2007  | Inaba et al.    | JP | 2006-53577  | 2/2006  |
| 2007/0196750 | A1 | 8/2007  | Fujiwara et al. | JP | 2006-79102  | 3/2006  |
| 2007/0212626 | A1 | 9/2007  | Toshine et al.  | JP | 3782680     | 3/2006  |
| 2008/0085459 | A1 | 4/2008  | Kami et al.     | JP | 3789081     | 4/2006  |
| 2008/0138725 | A1 | 6/2008  | Fujiwara et al. | JP | 2006-163302 | 6/2006  |
| 2008/0153021 | A1 | 6/2008  | Ikuno et al.    | JP | 2006-308743 | 11/2006 |
| 2008/0199217 | A1 | 8/2008  | Iwamoto et al.  | JP | 3878425     | 11/2006 |
| 2008/0227008 | A1 | 9/2008  | Kami et al.     | JP | 3878427     | 11/2006 |
| 2008/0311499 | A1 | 12/2008 | Kami et al.     | JP | 3878428     | 11/2006 |
| 2009/0067891 | A1 | 3/2009  | Kami et al.     | JP | 2007-79230  | 3/2007  |
| 2009/0148180 | A1 | 6/2009  | Fujiwara et al. | JP | 2007-79244  | 3/2007  |
| 2009/0208246 | A1 | 8/2009  | Kami            | JP | 2007-86319  | 4/2007  |

## FOREIGN PATENT DOCUMENTS

|    |             |         |    |             |         |
|----|-------------|---------|----|-------------|---------|
| JP | 5-88392     | 4/1993  | JP | 4011790     | 9/2007  |
| JP | 7-104497    | 4/1995  | JP | 2007-292772 | 11/2007 |
| JP | 7-292095    | 11/1995 | JP | 2008-70540  | 3/2008  |
| JP | 2509292     | 4/1996  | JP | 4110116     | 4/2008  |
| JP | 8-248663    | 9/1996  | JP | 2008-122869 | 5/2008  |
| JP | 3040540     | 3/2000  | JP | 4136567     | 6/2008  |
| JP | 2000-162881 | 6/2000  | JP | 4194973     | 10/2008 |
| JP | 2000-171990 | 6/2000  | JP | 4400704     | 11/2009 |
| JP | 2001-265014 | 9/2001  |    |             |         |
| JP | 2001-289630 | 10/2001 |    |             |         |
| JP | 2001-343771 | 12/2001 |    |             |         |
| JP | 2002-82468  | 3/2002  |    |             |         |
| JP | 2002-196645 | 7/2002  |    |             |         |
| JP | 2002-251029 | 9/2002  |    |             |         |
| JP | 2002-296994 | 10/2002 |    |             |         |
| JP | 2002-311613 | 10/2002 |    |             |         |

## OTHER PUBLICATIONS

“Measuring Non-Electrostatic Adhesive Force between Solid Surfaces and Particles by Means of Atomic Force Microscopy”, Mizuguchi et al., Konica Minolta Technology Report vol. 1 (2004) pp. 19-22.

FIG. 1



FIG. 2



FIG. 3



FIG. 4



FIG. 5



FIG. 6



FIG. 7



FIG. 8



FIG. 9A



FIG. 9B



FIG. 9C



FIG. 10



FIG. 11



FIG. 12



FIG. 13



FIG. 14



FIG. 15



FIG. 16



FIG. 17



FIG. 18



FIG. 19



FIG. 20



FIG. 21



FIG. 22



FIG. 23



FIG. 24



FIG. 25



FIG. 26



FIG. 27



FIG. 28



FIG. 29



FIG. 30



FIG. 31



FIG. 32



FIG. 33



FIG. 34



FIG. 35



FIG. 36



FIG. 37



FIG. 38



FIG. 39



FIG. 40



FIG. 41



FIG. 42



FIG. 43



FIG. 44



FIG. 45



FIG. 46



FIG. 47



## 1

**ELECTROPHOTOGRAPHIC  
PHOTORECEPTOR, METHOD OF  
MANUFACTURING  
ELECTROPHOTOGRAPHIC  
PHOTORECEPTOR, IMAGE FORMING  
APPARATUS, AND PROCESS CARTRIDGE**

**CROSS-REFERENCE TO RELATED  
APPLICATIONS**

This document claims priority from and contains subject matter related to Japanese Patent Applications Nos. 2009-061268 and 2010-046096, filed on Mar. 13, 2009 and Mar. 3, 2010, respectively, the entire contents of each of which are hereby incorporated herein by reference.

**BACKGROUND OF THE INVENTION**

**1. Field of the Invention**

The present invention relates to an electrophotographic photoreceptor for use in copiers, facsimile machines, laser printers, and direct digital platemakers. In addition, the present invention also relates to a method of manufacturing electrophotographic photoreceptor, and an image forming apparatus and a process cartridge using the electrophotographic photoreceptor.

**2. Discussion of the Related Art**

Recently, the mainstream of electrophotographic photoreceptor (hereinafter simply "photoreceptor") has switched from inorganic photoreceptor that uses inorganic materials such as selenium, zinc oxide, and cadmium sulfide, to organic photoreceptor that uses organic materials. Organic photoreceptors are more advantages than inorganic photoreceptors in reduction of environmental load and manufacturing cost and flexibility in compositional designing. Nowadays, the production of organic photoreceptors comes close to 100% of the total production of photoreceptors. Recently, organic photoreceptors are sought to be mechanical components rather than consumable supplies in accordance with increasing momentum of global environmental protection.

Various attempts have been made to improve durability of organic photoreceptors. For example, Japanese Patent Application Publication No. (hereinafter "JP-A") 2000-66424 and JP-A 2000-171990 have proposed forming a cross-linked resin layer and a zol-gel cured resin layer, respectively, on the surface of a photoreceptor. The former is more productive because the layer is likely to neither fracture nor crack even when an electron transport material is added thereto. In particular, radical-polymerized acrylic resins are advantages because of having high stiffness and providing the resultant photoreceptor with high photosensitivity. Because of including plural chemical bonds, such cross-linked or cured resin layers may not be immediately brought into abrasion even when a part of chemical bonds are cut by application of mechanical stress.

On the other hand, the mainstream of electrophotographic toner (hereinafter simply "toner") is switching from irregular-shaped toner to spherical toner. Spherical toners have an advantage in production of high quality image.

Generally, spherical toners are manufactured by chemical manufacturing methods such as a suspension polymerization method, an emulsion aggregation polymerization method, an ester elongation method, and a dissolution suspension method. Spherical toners may be hereinafter referred to as "polymerization toners" as appropriate. For example, a typical polymerization toner for use in an electrophotographic image forming apparatus may have an average circularity of

## 2

from 0.95 to 0.99 and shape factors SF-1 and SF-2 of from 110 to 140. A true sphere has a circularity of 1.0 and shape factors of 100.

Because of having a uniform shape, each polymerization toner particles has a uniform charge quantity. Therefore, polymerization toner particles develop a latent image into a toner image with high sharpness, resolution, and gradation. In addition to this high developability, polymerization toner particles also have high transfer efficiency. Also, because polymerization toner particles are easy to include wax, advantageously, oil is not needed when fixed on recording media such as paper.

At the same time, disadvantageously, polymerization toner particles are difficult to be removed when remaining on a photoreceptor. To solve this problem, a greater amount of external additives are required on the surfaces of the polymerization toner particles. As a result, the external additives may form undesired films thereof on the photoreceptor.

In order to more effectively remove residual polymerization toner particles from a photoreceptor, one proposed approach involves applying a solid lubricant (e.g., zinc stearate) to a surface of a photoreceptor to reduce the surface friction coefficient thereof, as described in a technical document entitled "Blade cleaning system for polymerized and small size toner, Hyakutake et al., Japan Hardcopy Fall Meeting, 2001, 24-27".

However, a solid lubricant (e.g., zinc stearate) may not be sufficiently applied to a surface of a photoreceptor when the surface is relatively smooth.

In view of this, JP-A 2007-79244 proposed to roughen a surface of a photoreceptor so that a lubricant is reliably applied thereto, in other words, receptivity of the surface to a lubricant is improved. It is disclosed therein that a surface of a photoreceptor preferably has a surface roughness Rz (defined in JIS B0601-1994) of from 0.4 to 1.0  $\mu\text{m}$ , which can be achieved by addition of a filler to the surface layer.

Although having the same Rz value, the surface profile of a photoreceptor may vary. For example, even when the average distance between the highest peak and lowest valley is extremely different, the Rz value may be the same. Therefore, receptivity of the surface to zinc stearate may not be improved only by controlling the Rz value.

In addition to Rz (ten points average roughness), Ra (arithmetical average roughness), Rmax (the maximum height), etc., all defined in JIS B0601, are also widely used for evaluation of surface roughness. However, these parameters are not satisfactory to evaluate surface roughness of photoreceptors, and various proposals have been made as follows.

JP-A 07-104497 discloses a method in which a divisional breadth X having an average line 2 at center is assumed on a cross section curve 1 obtained through the measurement of surface contour with a surface roughness measuring device, and the surface contour is evaluated on the basis of the number of peaks 4 of a pair of adjacent crest and trough outside the breadth X per unit length L. In this case, a substrate having the number of the peaks 4 equal to or less than 100 with the breadth X kept at 20  $\mu\text{m}$  and the unit length L at 1 cm is used to fabricate an organic photoreceptor.

To form high quality image by solving the problem of insufficient cleaning of small-size toner, JP-A 2002-196645 discloses an image forming device in which a cleaning roll having bias voltage applied to separate electrified toner from a photoreceptor is provided on the upstream side of a cleaning blade, and a photoreceptor having a surface roughness Rz of 0.1  $\mu\text{m}$  to 2.5  $\mu\text{m}$  in an average of ten points is provided.

JP-A 2006-163302 discloses an electrophotographic photoreceptor which satisfies  $\Delta T > Rz$  and  $0 \mu\text{m} < \Delta T + Rz < 5 \mu\text{m}$ ,

wherein  $\Delta T$  and  $Rz$  represent the wear amount and the surface roughness, respectively, per kilecycle of the electrophotographic photoreceptor.

JP-A 2007-86319 discloses an electrophotographic photoreceptor in which the surface of the photosensitive layer is subjected to surface roughening treatment, and when the glossiness of the surface of the photosensitive layer after the surface roughening treatment is measured, a standard deviation of the measurement value is  $\leq 4$ .

Japanese Patent No. 3040540 (corresponding to JP-A 04-243265) discloses an image forming system which includes a blade, an image forming member, and a toner composition. The image forming member has a surface on which the toner composition forms an image, and the surface has surface roughnesses defined by the following inequations:

$$R/ann^4 > KB(1-\sigma^2)/32\pi E^2 a^2$$

$$R/ann^2 > \sqrt{3}/8\pi^2 \cdot (1+\mu^2) \cdot \mu \cdot KB/\Gamma \cdot t/a^2$$

wherein  $R$  is the average height of the projecting parts of the surface;  $ann$  is half the nearest adjacent distance between the projecting parts on the surface;  $KB$  is the bulk elastic modulus of the blade;  $\sigma$  is the Poisson's ratio of the toner composition;  $E$  is the Young's modulus of the toner composition;  $t$  is the average thickness of flat particles in the toner composition;  $a$  is the average radius of the flat particles;  $\mu$  is the average between the coefficient of friction of the toner blade and the coefficient of friction of toner surfaces;  $\Gamma$  is the Dupre' work of the adhesion between the surface and the flat particles; and  $\theta$  is a blade tip angle.

Japanese Patent No. 3938209 (corresponding to WO 05/093518) discloses a cylindrical electrophotography photosensitive body having a cylindrical support and an organic photosensitive layer provided on the cylindrical support. The circumferential surface of the electrophotography photosensitive body has recesses of dimple shape. The ten point average height  $Rz_{jis}$  (A) measured by scanning in the circumferential direction of the circumferential surface of the electrophotography photosensitive body is 0.3 to 2.5  $\mu\text{m}$ , and the ten point average height  $Rz_{jis}$  (B) measured by scanning in the direction of the generating line of the circumferential surface of the electrophotography photosensitive body is 0.3 to 2.5  $\mu\text{m}$ . The average interval  $RSm$  (C) of the irregularities measured by scanning in the circumferential direction of the circumferential surface of the electrophotography body is 5 to 120  $\mu\text{m}$ , and the average interval  $RSm$  (D) of the irregularities measured by scanning in the direction of the generating line of the circumferential surface of the electrophotography photosensitive body is 5 to 120  $\mu\text{m}$ . The ratio (D/C) of the average interval  $RSm$  (D) of the irregularities to the average interval  $RSm$  (C) of the irregularities is 0.5 to 1.5.

Japanese Patent No. 3938210 (corresponding to WO 05/093520) discloses an electrophotographic photosensitive member having a support and an organic photosensitive layer provided on the support. A plurality of dimple-shaped concavities are formed on the surface of the surface layer of the electrophotographic photosensitive member and a plurality of recesses corresponding to the dimple-shaped concavities formed on the surface of the surface layer are formed on the interface between the surface layer and a layer directly under the surface layer.

JP-A 2005-345788 discloses an image forming apparatus having a plurality of image carriers which are each obtained by disposing a photosensitive layer on a conductive support and on which electrostatic latent images are formed by surface exposure, a plurality of development devices, and a plu-

rality of cleaning means. At least a pair of development devices among a plurality of developing devices house developers having the same hue but different from each other in luminosity. The compositions or physical values of surface layers of the image carriers are set according to the luminosity of the developers housed in the plurality of development devices.

JP-A 2004-258588 discloses an image forming apparatus including a photoreceptor having a surface performance that the ten-point average roughness  $Rz_{jis}$  is  $\geq 0.1 \mu\text{m}$  and  $\leq 1.5 \mu\text{m}$  or the maximum height  $Rz$  is 2.5  $\mu\text{m}$  or less, and the frictional resistance  $Rf$  is  $\geq 45 \text{ gf}$  and  $\leq 200 \text{ gf}$ .

JP-A 2004-054001 discloses an image forming method including a primary transferring process transferring a toner image visualized by developing onto an intermediate transfer body, a secondary transferring process transferring the toner image transferred onto the intermediate transfer body onto a recording medium, and a cleaning process in which residue toner on an electrophotographic photoreceptor is eliminated after transferring the toner image onto the recording material. The surface roughness  $Ra$  of the electrophotographic photoreceptor is 0.02 to 0.1  $\mu\text{m}$ , the surface roughness  $Rz$  of the intermediate transfer body is 0.4  $\mu\text{m}$  to 2.0  $\mu\text{m}$ , and image formation is carried out by feeding surface energy lowering agent to the surface of the electrophotographic photoreceptor.

JP-A 2003-270840 discloses an image forming apparatus including an organic photoreceptor in which the average cycle of the surface irregularity is 10 times or more the volume average particle diameter of the toner used therefor.

JP-A 2003-241408 discloses an electrophotographic device including an electrophotographic photoreceptor rotating at a peripheral speed of 200 mm/sec or more and a cleaning means. The electrophotographic photoreceptor has a photosensitive layer and a surface protection layer on a conductive base. The surface protection layer contains 35.0 to 45.5 mass % fluorine atom containing resin particles for the total mass of the protection layer and is of 0.1 to 5.0  $\mu\text{m}$  in 10-point mean surface roughness, 0.1 to 10.0 in surface hardness by a Taber's abrasion resistant test method, and 0.1 to 0.7 in surface friction coefficient. The cleaning means is a rubber elastic body blade and the linear pressure of the blade to the electrophotographic photoreceptor is 0.294 to 0.441 N/cm. The glass transition point ( $T_g$ ) of toner in use is 40 to 55°C. The tensile modulus (Young's modulus) as a blade property value is 784 to 980 N/cm<sup>2</sup>. The value of repulsive elasticity is 35 to 55%. Fluorine atom resin particulates are incorporated in the surface of the base material.

JP-A 2003-131537 discloses an image forming method including an image forming body on which a toner forms an image, which satisfies the equation  $d/t \times 0.01 \leq Ra \leq 0.5$ , wherein  $d/t$  represents the degree of flatness of the toner particle ( $d$  represents the volume average particle diameter of the toner and  $t$  represents the thickness  $t$  of the toner particle) and  $Ra$  ( $\mu\text{m}$ ) represents a surface roughness of the image forming body.

JP-A 2002-296994 and JP-A 2002-258705 each disclose an image forming apparatus including an image bearing member on which a spherical toner forms an image, the surface of which has convexities and concavities which are smaller than the volume average particle of the toner.

JP-A 2002-082468 discloses an electrophotographic device having an electrophotographic photoreceptor which is rotated above 200 mm/sec in circumferential speed and a cleaning means. The photoreceptor has a photosensitive layer and a surface protective layer on a conductive substrate. The surface protective layer contains 15.0 to 40.0 mass % fluorine atom-containing resin particles. Its surface roughness is 0.1 to

5.0  $\mu\text{m}$  in ten-point mean roughness, its surface hardness is 0.1 to 20.0 in a taper wear test method, and its surface friction coefficient is 0.001 to 1.2.

JP-As 2001-265014, 2001-289630, 2002-251029, 2002-296822, 2002-296823, 2002-296824, 2002-341572, 2006-53576, 2006-53577, and 2006-79102 disclose methods of evaluating surface profile using Fourier transform. In Fourier transform, a variation which occurs with high frequency in a signal can be transformed into a frequency distribution, however, a variation which occurs with low frequency cannot. Further, disadvantageously, it is not clearly determined from the results of Fourier transform where the variation occurred.

JP-A 2004-117454 discloses a method for evaluating the surface roughness of a base body for an electrophotographic photoreceptor. A cross section curve stipulated by JIS B0601 from an arbitrary position of the base body surface is obtained in the abscissa direction by a length of 100  $\mu\text{m}$ , positions of the cross section curve in the ordinate direction at equispaced positions in the abscissa direction are measured, variance of the positions stipulated by JIS Z8101 is obtained, one or more measurements selected from surface roughnesses Ra, Rz and Ry stipulated by JIS B0601 are also obtained, and the surface roughness of the base body is evaluated using the variance and the one or more measurements.

JP-A 2004-61359 discloses a surface roughness evaluating method of a component for an image forming device. A cross-section curve defined by JIS B0601 is found on the surface condition of the component to perform multiple resolution analysis on positional data rows in a surface roughness direction at equally spaced positions on the cross-section curve, and the state of the surface roughness is evaluated at least based on the result.

JP-A 2007-292772 discloses a surface roughness evaluating method of a component for an image forming device. A profile curve defined in JIS B0601 is calculated on a surface condition of the image forming apparatus component such as the electrophotographic photoreceptor substratum. Multiple resolution analysis such as wavelet transformation of a positional data row in the surface roughness direction at equal intervals on the profile curve is performed, and the surface roughness condition is evaluated based on the results.

JP-A 2008-70540 discloses a latent electrostatic image bearing member having a cross-linked surface layer which comprises a reactive silicone material. It is disclosed therein that such a surface layer is smooth and has a low surface energy, providing good cleanability of toners.

However, none of the above-described methods of evaluating surface roughness is sufficient to evaluate cleanability (removability) of small-size toners and polymerization (spherical) toners from photoreceptor.

In view of this situation, surface roughness may be evaluated from a surface profile recorded on a chart by a surface roughness & profile shape measuring instrument. However, it requires skill to evaluate surface roughness from the chart.

Namely, any of the parameters (Ra, Rmax, Rz, etc.) does not sufficiently represent cleanability (removability) of small-size toners and polymerization (spherical) toners from photoreceptor.

In the above-cited reference JP-A 2007-79244, a photoreceptor including alumina particles as a filler is disclosed. Since alumina particles are difficult to be uniformly dispersed in a coating material, it requires a special technique to form a uniform coating layer. A photoreceptor including polymethylsilsesquioxane particles is also disclosed therein. Such a photoreceptor does not always sufficiently hold a solid lubricant hereon because of having too large convexities and concavities on the surface thereof.

Although a coating material for forming a cross-linked resin surface layer has a low viscosity because of being comprised primarily of monomer components, silicon-containing particles such as silica particles and silicone resin particles can be stably dispersed therein. Accordingly, silicon-containing particles have a great advantage over various filler materials in manufacturing photoreceptors. However, silicon-containing particles do not always provide the resultant photoreceptor with high receptivity to solid lubricants, as seen in Example 2 of JP-A 2005-99688. This is because the surface of the photoreceptor has too large convexities and concavities to hold solid lubricants.

JP-A 08-248663 discloses a photoreceptor in which a photosensitive layer is provided on a conductive base. Surface roughness of the conductive base is 0.01-2.0  $\mu\text{m}$  while surface roughness of the outermost surface side layer is 0.1-0.5  $\mu\text{m}$ . And in the outermost surface side layer, inorganic grains with an average grain diameter of 0.05-0.5  $\mu\text{m}$  are contained.

As described therein, the inorganic grain such as silica particle may be hydrophobized in an attempt to improve durability and prevent deterioration of image resolution which occurs by adhesion of contaminants such as corona products. However, the hydrophobized inorganic grain may not prevent adhesion of corona products while preventing adhesion of water, thereby causing image blurring.

In view of this situation, JP-A 2004-138643 proposed to use alumina as a filler to prevent image blurring. However, a special technique is required to disperse alumina in a cross-linked resin surface layer, as described above.

As seen above, the receptivity of a photoreceptor to solid lubricants may affect abrasion rate of the photoreceptor and/or cleanability (removability) of toner, i.e., printing quality. However, any technique to improve the receptivity of a highly-durable photoreceptor having a cross-linked resin surface layer has not been proposed so far.

Advantageously, such a photoreceptor having a surface layer such as a cross-linked resin layer has extremely high durability. On the other hand, disadvantageously, such a surface layer has a low receptivity to solid lubricants and therefore cleanability (removability) of polymerization toners is poor. As a result, highly-durable photoreceptors having a surface layer cannot be practically used in combination with polymerization toners under the current situation.

## SUMMARY OF THE INVENTION

Accordingly, exemplary embodiments of the present invention provide an electrophotographic photoreceptor having good receptivity to solid lubricants, a method of manufacturing such an electrophotographic photoreceptor having good receptivity to solid lubricants, and an image forming apparatus and a process cartridge having a long lifespan.

These and other features and advantages of the present invention, either individually or in combinations thereof, as hereinafter will become more readily apparent can be attained by exemplary embodiments described below.

One exemplary embodiment provides an electrophotographic photoreceptor including a conductive substrate, a photosensitive layer located overlying the conductive substrate, and a surface layer located overlying the photosensitive layer. The electrophotographic photoreceptor satisfies the following inequations:

$$0.005 < WRa(LMH) < 0.03 \quad (i)$$

$$0.010 < WRa(LHH) < 0.03 \quad (ii)$$

$$0.005 < WRa(LML) < 0.20 \quad (iii)$$

WRa(LLH)&gt;WRa(LMH)

(iv)

WRa(LLH)&gt;WRa(LHH)

(v)

wherein WRa ( $\mu\text{m}$ ) represents a center-line average roughness of frequency components LHH, LHL, LMH, LML, LLH, and LLL that are obtained by: subjecting a one-dimensional data array of a surface profile of the electrophotographic photoreceptor, which is measured with a surface roughness & profile shape measuring instrument, to wavelet transformation multiresolution analysis so as to be separated into 6 frequency components each having a cycle length ( $\mu\text{m}$ ) of 0 to 3, 1 to 6, 2 to 13, 4 to 25, 10 to 50, and 24 to 99; thinning a one-dimensional data array of the lowest frequency component having a cycle length of from 24 to 99 ( $\mu\text{m}$ ) so that the number of data array is reduced to 1/40; and subjecting the thinned one-dimensional data array to wavelet transformation multiresolution analysis so as to be separated into the 6 frequency components LHH, LHL, LMH, LML, LLH, and LLL each having a cycle length ( $\mu\text{m}$ ) of 26 to 106, 53 to 183, 106 to 318, 214 to 551, 431 to 954, and 867 to 1,654, respectively.

Another exemplary embodiment provides a method of manufacturing electrophotographic photoreceptor including coating and curing a surface layer coating liquid on a photo-sensitive layer. The surface layer coating liquid may be either a cross-linked resin surface layer coating liquid or a thermo-plastic resin surface layer coating liquid.

Yet another exemplary embodiment provides an image forming apparatus including the above-described electrophotographic photoreceptor configured to bear an electrostatic latent image, a brush roller configured to apply a solid lubricant to a surface of the electrophotographic photoreceptor, a blade configured to extend the solid lubricant on the surface of the electrophotographic photoreceptor, and a developing device configured to develop the electrostatic latent image with a toner to form a toner image.

Yet another exemplary embodiment provides a process cartridge detachably mountable on image forming apparatus, including the above-described electrophotographic photoreceptor configured to bear an electrostatic latent image, a brush roller configured to apply a solid lubricant to a surface of the electrophotographic photoreceptor, and a blade configured to extend the solid lubricant on the surface of the electrophotographic photoreceptor.

#### BRIEF DESCRIPTION OF THE DRAWINGS

A more complete appreciation of the embodiments described herein and many of the attendant advantages thereof will be readily obtained as the same becomes better understood by reference to the following detailed description when considered in connection with the accompanying drawings, wherein:

FIG. 1 is a schematic view illustrating an example embodiment of a lubricant applicator;

FIGS. 2 to 7 are schematic views illustrating various application conditions of a solid lubricant to a photoreceptor;

FIG. 8 is a schematic view illustrating an example embodiment of a surface profile evaluating device;

FIGS. 9A to 9C show example results of the wavelet transformation multiresolution analysis;

FIG. 10 is a graph showing frequency bands separated in the first multiresolution analysis;

FIG. 11 is the result of the thinning treatment of the curve 106 (HLL) in FIG. 9;

FIG. 12 is a graph showing frequency bands separated in the second multiresolution analysis;

FIG. 13 is a schematic view illustrating an embodiment of the photoreceptor of the present invention;

FIG. 14 is a schematic view illustrating another embodiment of the photoreceptor of the present invention;

FIG. 15 is a schematic view illustrating an embodiment of the image forming unit;

FIG. 16 is a schematic view illustrating another embodiment of the image forming unit;

FIG. 17 is a schematic view illustrating an embodiment of the process cartridge of the present invention;

FIG. 18 is a schematic view illustrating another embodiment of the image forming unit;

FIG. 19 is a schematic view illustrating another embodiment of the image forming unit;

FIG. 20 is a schematic view illustrating another embodiment of the image forming unit;

FIG. 21 is a schematic view illustrating an embodiment of the solid lubricant applicator;

FIG. 22 is a schematic view illustrating a color copier used in a solid lubricant receptivity test;

FIG. 23 is an example result of the image analysis in the solid lubricant receptivity test; and

FIGS. 24 to 47 are measurement results of WRa in Examples and Comparative Examples.

#### DESCRIPTION OF THE PREFERRED EMBODIMENTS

First, a general application mechanism of a solid lubricant to a surface of a photoreceptor in an electrophotography is described in detail.

A lubricant in a powder state is applied to a surface of a photoreceptor in a small amount. More specifically, for example, a block-shaped solid lubricant is scraped with a brush-shaped applicator and is applied to a surface of a photoreceptor, as described in JP-A 2000-162881, the disclosure thereof being incorporated herein by reference. Such a procedure can be performed by a simple apparatus and is able to reliably apply a lubricant to the entire surface of a photoreceptor.

FIG. 1 is a schematic view illustrating an example embodiment of a lubricant applicator. An application brush 3B, such as a fur brush, rotates so as to scrape a solid lubricant 3A and apply it to a photoreceptor 31. The application brush 3B rotates while contacting the solid lubricant 3A so that a part of the solid lubricant 3A is scraped off. The scraped solid lubricant 3A adheres to the application brush 3B, and the application brush 3B applies the scraped solid lubricant 3A to the photoreceptor 31 by rotation. Because the scraped solid lubricant 3A that is in a powder state may not express lubricity, the scraped solid lubricant 3A is drawn or extended with an application blade 39 to form a thin film thereof on the photoreceptor 31.

The solid lubricant 3A may be a higher fatty acid metal salt such as zinc stearate, for example. Zinc stearate is a lamella crystal, which is preferably used as the lubricant. Lamella crystals generally have a layered structure in which amphiphilic molecules are self-assembled, and easily fracture along the interfaces between the layers upon application of shear force. Accordingly, a lamella crystal may cover the entire surface of a photoreceptor upon application of shear force to reduce the friction coefficient even in a small amount.

There are various methods of controlling lubricant application conditions. One example method includes increasing the contact pressure of the solid lubricant 3A with the application brush 3B. Another example method includes controlling the revolution speed of the application brush 3B.

The surface roughness of a photoreceptor cannot be satisfactorily controlled only by monitoring conventional parameters such as Ra and RSm which are measureable with a surface roughness & profile shape measuring instrument, as described above. In view of this situation, the inventors of the present invention found that the surface roughness of a photoreceptor can be satisfactorily controlled by wavelet transformation multiresolution analysis of a one-dimensional data array of a cross-sectional curve of the photoreceptor.

More specifically, the inventors of the present invention found that there is a relation between application conditions of a solid lubricant and a center-line average roughness WRa of a photoreceptor. In the present specification, the center-line average roughness WRa is calculated as follows. First, a one-dimensional data array of a surface profile of a photoreceptor measured with a surface roughness & profile shape measuring instrument is subjected to wavelet transformation multiresolution analysis so as to be separated into plural frequency components, ranging from high-frequency components to low-frequency components. A one-dimensional data array of the lowest-frequency component is thinned and further subjected to wavelet transformation multiresolution analysis so as to be separated into plural frequency components. Each of the frequency components are subjected to calculation of the center-line average roughness WRa, based on a method of calculating the center-line average roughness Ra that is defined in JIS B0601-1982.

Accordingly, an exemplary embodiment of the present invention provides an electrophotographic photoreceptor including a conductive substrate, a photosensitive layer located overlying the conductive substrate, and a surface layer located overlying the photosensitive layer, which satisfies the following inequations:

$$0.005 < WRa(LMH) < 0.03 \quad (i)$$

$$0.010 < WRa(LHH) < 0.03 \quad (ii)$$

$$0.005 < WRa(LML) < 0.20 \quad (iii)$$

$$WRa(LLH) > WRa(LMH) \quad (iv)$$

$$WRa(LLH) > WRa(LHH) \quad (v)$$

wherein WRa ( $\mu\text{m}$ ) represents a center-line average roughness of frequency components LHH, LHL, LMH, LML, LLH, and LLL that are obtained by: subjecting a one-dimensional data array of a surface profile of the electrophotographic photoreceptor, which is measured with a surface roughness & profile shape measuring instrument, to wavelet transformation multiresolution analysis so as to be separated into 6 frequency components each having a cycle length ( $\mu\text{m}$ ) of 0 to 3, 1 to 6, 2 to 13, 4 to 25, 10 to 50, and 24 to 99; thinning a one-dimensional data array of the lowest frequency component having a cycle length of from 24 to 99 ( $\mu\text{m}$ ) so that the number of data array is reduced to 1/40; and subjecting the thinned one-dimensional data array to wavelet transformation multiresolution analysis so as to be separated into the 6 frequency components LHH, LHL, LMH, LML, LLH, and LLL each having a cycle length ( $\mu\text{m}$ ) of 26 to 106, 53 to 183, 106 to 318, 214 to 551, 431 to 954, and 867 to 1,654, respectively.

When the inequations (i) to (v) are satisfied, a solid lubricant is applied to the surface layer in very good condition. The reason for this may be considered that the surface profile of the surface layer matches the application mechanism of the solid lubricant.

Photoreceptors are generally required to be sensitive to adhesion of solid lubricants. Such a sensitivity of photorecep-

tors to adhesion of solid lubricants may be influenced by 1) the adhesion force between a photoreceptor and a solid lubricant and/or 2) the ease of formation of a thin film of a solid lubricant with an application blade.

For example, the adhesion force between two substances is studied in a technical document entitled "Measuring Non-Electrostatic Adhesive Force between Solid Surfaces and Particles by Means of Atomic Force Microscopy, Mizuguchi et al., KONICA MINOLTA TECHNOLOGY REPORT VOL. 1 (2004), 19-22". It is considered therein that the adhesion force between two substances is influenced by non-electrostatic attraction force, electrostatic attraction force, and the contact area therebetween. The electrostatic attraction force may be generated from a contact potential difference. The non-electrostatic attraction force may be generated from a difference in surface energy (e.g., wettability).

Generally, solid lubricants have low adhesive property. Therefore, the adhesion force between a solid lubricant and a photoreceptor is unlikely to drastically increase even if various surface controlling agents are included in the surface of the photoreceptor. In view of this situation, the inventors of the present invention focused on the contact area therebetween.

FIGS. 2 to 7 are schematic views illustrating various application conditions of a solid lubricant to a photoreceptor. As illustrated in FIG. 2, the solid lubricant 3A adhering to the photoreceptor 31 is in the form of a powder, an aggregation, or a solid block. When the surface of the photoreceptor 31 is smooth as illustrated in FIG. 3, the solid lubricant 3A cannot pass through an edge 3D of the application blade 39 and sideslips on the photoreceptor 31, and consequently releases from the surface of the photoreceptor 31. By contrast, when the surface of the photoreceptor 31 has an extreme irregularity as illustrated in FIG. 4, the solid lubricant 3A point-contacts the photoreceptor 31 and consequently releases from the surface of the photoreceptor 31 as well.

When the irregularity is not cyclic, sideslip of the solid lubricant 3A is prevented. However, in this case, an aggregation of the solid lubricant 3A point-contacts an edge of a convexity or concavity, as illustrated in FIG. 5, and consequently releases from the surface of the photoreceptor 31 as well.

When the surface has a gentle irregularity as illustrated in FIG. 6, the solid lubricant 3A may pass through the edge 3D of the application blade 39 or may be extended on the surface of the photoreceptor 31, depending on the linear pressure of the application blade 39. When a high-frequency irregularity is further superimposed on the gentle irregularity that prevents sideslip of the solid lubricant 3A, as illustrated in FIG. 7, the solid lubricant 3A more strongly adheres to the photoreceptor 31. Namely, when the following inequations are satisfied, it means that the surface has a gentle (i.e., low-frequency) irregularity so that the solid lubricant 3A is extended thereon:

$$0.005 < WRa(LML) < 0.20$$

$$0.005 < WRa(LMH) < 0.03$$

and when the following inequation is satisfied, it means that the surface has a high-frequency irregularity so that the solid lubricant 3A strongly adheres thereto:

$$0.010 < WRa(LHH) < 0.03$$

A procedure for measuring WRa is described in detail below.

First, a surface of a photoreceptor is subjected to a measurement of a one-dimensional data array of a primary profile that is defined in JIS B0601.

## 11

The one-dimensional data array may be a digital signal directly obtained from a surface roughness & profile shape measuring instrument or that obtained by analog-digital conversion of an analog output of a surface roughness & profile shape measuring instrument.

According to JIS B0601, the evaluation length is preferably from 8 to 25 mm.

The sampling length is preferably 1  $\mu\text{m}$  or less, and more preferably from 0.2 to 0.5  $\mu\text{m}$ .

For example, when the evaluation length is 12 mm and the number of sampling points is 30,720, the sampling length becomes 0.390625  $\mu\text{m}$ , which is within the above preferable range.

The one-dimensional data array is subjected to wavelet transformation multiresolution analysis so as to be separated into plural frequency components, ranging from high-frequency components to low-frequency components. A one-dimensional data array of the lowest-frequency component is thinned and further subjected to wavelet transformation multiresolution analysis so as to be separated into plural frequency components. The center-line average roughness W<sub>RA</sub> is calculated from each of the frequency components based on a method of calculating the center-line average roughness R<sub>a</sub> that is defined in JIS B0601-1982.

As described above, wavelet transformation multiresolution analysis is performed twice. For the sake of simplicity, the first and second wavelet transformation multiresolution analysis may be hereinafter represented as MRA-1 and MRA-2, respectively. The frequency components are distinguished by prefixes H and L indicating the results of the first and second wavelet transformation, respectively.

Mother wavelet functions usable for the first and second wavelet transformation may be the Daubecies function, Harr function, Meyer function, Symlet function, or Coiflet function, for example. In the present embodiment, the Harr function is used as the mother wavelet function.

As a result of the wavelet transformation multiresolution analysis, the number of resultant frequency components is preferably from 4 to 8. In the present embodiment, the number of resultant frequency components is 6.

In the first wavelet transformation, a one-dimensional data array is separated into plural frequency components. Another one-dimensional data array is created from the lowest-frequency component and is thinned. The thinned one-dimensional data array is subjected to the second wavelet transformation so as to be separated into plural frequency components.

The lowest-frequency component obtained in the first wavelet transformation is thinned so that the number of data array is reduced to from  $1/10$  to  $1/100$ . In other words, the thinning factor is from  $1/10$  to  $1/100$ .

Such a thinning treatment of data increases the frequency of data. For example, when a one-dimensional data array including 30,000 data arrays obtained in the first wavelet transformation is thinned so that the number of data arrays is reduced to  $1/10$ , the thinned one-dimensional data array includes 3,000 data arrays.

When the thinning factor is less than  $1/10$ , for example,  $1/5$ , the frequency of data may not increase. In this case, the second wavelet transformation multiresolution analysis may result in insufficient data separation.

When the thinning factor is greater than  $1/100$ , for example,  $1/200$ , the frequency of data may increase too much. In this case, the second wavelet transformation multiresolution analysis may result in insufficient data separation such that the resulting frequency components concentrate at high frequencies.

## 12

In the present embodiment, the thinning factor is  $1/40$ .

FIG. 8 is a schematic view illustrating an example embodiment of a surface profile evaluating device. In FIG. 8, a numeral 41 denotes a photoreceptor, a numeral 42 denotes a jig equipped with a probe for measuring surface roughness, a numeral 43 denotes a unit for moving the jig 42 along a measuring object, a numeral 44 denotes a surface roughness & profile shape measuring instrument, and a numeral 45 denotes a personal computer for analyzing data signals. The personal computer 45 performs the multiresolution analysis. When the photoreceptor 41 has a cylindrical shape, the measurement can be performed both in the peripheral and longitudinal directions.

The embodiment of the surface profile evaluation device is not limited to that illustrated in FIG. 8. For example, the multiresolution analysis may be performed by a numerical calculation processor. Alternatively, the multiresolution analysis may be performed by the surface roughness & profile shape measuring instrument itself.

The analysis results may be displayed on a CRT or a liquid crystal display or may be print-outputted. Alternatively, the analysis results may be transmitted to another device as electric signals or stored on a USB memory or a MO disc.

In the present embodiment, a surface texture and contour measuring instrument SURFCOM 1400D (from Tokyo Seimitsu Co., Ltd.) is used as the surface roughness & profile shape measuring instrument 44 and a personal computer from IBM is used as the personal computer 45, and the SURFCOM 1400D and the personal computer are connected with RS-232-C cable. Surface roughness data is transmitted from the SURFCOM 1400D to the personal computer and is subjected to data processing and multiresolution analysis using a software program written in C language by the inventors of the present invention.

The procedure for the multiresolution analysis of a surface profile of a photoreceptor is described in detail below.

First, a primary profile of a photoreceptor is measured with a surface texture and contour measuring instrument SURFCOM 1400D (from Tokyo Seimitsu Co., Ltd.). The evaluation length per measurement is 12 mm. The total number of sampling points is 30,720, and 4 sampling points are measured per measurement. The measurement results are transmitted to a personal computer and subjected to the first wavelet transformation with a software program written by the inventors. The lowest-frequency component is subjected to a thinning treatment with a thinning factor of  $1/40$ , and then subjected to the second wavelet transformation.

The resultant curves of the first and second multiresolution analysis are subjected to calculation of the center-line average roughness R<sub>a</sub>, maximum height, R<sub>max</sub>, and ten points average roughness R<sub>z</sub> according to JIS B0601-1982. FIGS. 9A to 9C show example results of the wavelet transformation multiresolution analysis.

In FIGS. 9A to 9C, the vertical axes are displacement scales ( $\mu\text{m}$ ) of surface profile. The lateral axes are evaluation length scales. In the present embodiment, the evaluation length is 12 mm.

FIG. 9A is a primary profile obtained with the SURFCOM 1400D. Conventionally, the center-line average roughness R<sub>a</sub>, maximum height, R<sub>max</sub>, and ten points average roughness R<sub>z</sub> according to JIS B0601-1982 are calculated only from this primary profile.

FIG. 9B shows 6 frequency components obtained in the first multiresolution analysis. A curve 101 is the highest-frequency component and a curve 106 is the lowest-frequency component.

The curve 101 is the highest-frequency component having a frequency of from 0 to 3  $\mu\text{m}$  obtained in the first multiresolution analysis, which may be hereinafter represented as HHH.

The curve 102 is the second highest-frequency component having a frequency of from 1 to 6  $\mu\text{m}$  obtained in the first multiresolution analysis, which may be hereinafter represented as HHL.

The curve 103 is the third highest-frequency component having a frequency of from 2 to 13  $\mu\text{m}$  obtained in the first multiresolution analysis, which may be hereinafter represented as HMH.

The curve 104 is the fourth highest-frequency component having a frequency of from 4 to 25  $\mu\text{m}$  obtained in the first multiresolution analysis, which may be hereinafter represented as HML.

The curve 105 is the fifth highest-frequency component having a frequency of from 10 to 50  $\mu\text{m}$  obtained in the first multiresolution analysis, which may be hereinafter represented as HLH.

The curve 106 is the lowest-frequency component having a frequency of from 24 to 99  $\mu\text{m}$  obtained in the first multiresolution analysis, which may be hereinafter represented as HLL.

The primary profile illustrated in FIG. 9A is separated into 6 curves that are illustrated in FIG. 9B based on the frequency.

FIG. 10 is a graph showing frequency bands separated in the first multiresolution analysis. The lateral axis represents the number of peaks and valleys per 1 mm when assuming a profile as a sine curve. The vertical axis represents the ratio of each of the frequency bands.

In FIG. 10, a curve 121 is a band of the highest-frequency component in the first multiresolution analysis. A curve 122 is a band of the second highest-frequency component in the first multiresolution analysis. A curve 123 is a band of the third highest-frequency component in the first multiresolution analysis. A curve 124 is a band of the fourth highest-frequency component in the first multiresolution analysis. A curve 125 is a band of the fifth highest-frequency component in the first multiresolution analysis. A curve 126 is a band of the lowest-frequency component in the first multiresolution analysis.

FIG. 10 indicates that when the number of peaks and valleys per 1 mm is 20 or less, it appears in the curve 126 only.

When the number of peaks and valleys per 1 mm is 110, it most strongly appears in the curve 124 corresponding to the curve 104 (HML) in FIG. 9B.

When the number of peaks and valleys per 1 mm is 220, it most strongly appears in the curve 123 corresponding to the curve 103 (HMH) in FIG. 9B.

When the number of peaks and valleys per 1 mm is 310, it appears in the curves 122 and 123 corresponding to the curves 102 (HHL) and 103 (HM), respectively, in FIG. 9B.

It depends on the frequency of a surface roughness in which curve in FIG. 9B it may appear.

In other words, relatively fine irregularities appear in the curves in the upper side of FIG. 9B while relatively coarse irregularities appear in the curves in the lower side of FIG. 9B.

Namely, a surface profile measured with a surface roughness & profile shape measuring instrument is separated into the plural curves 101 to 106 based on the frequency, as illustrated in FIG. 9B. Therefore, the number of peaks and valleys in each frequency band can be separately measured.

The curves 101 to 106 are further subjected to the calculation of the center-line average roughness Ra, maximum

height, Rmax, and ten points average roughness Rz according to JIS B0601-1982. The calculated values thereof are shown in FIG. 9B.

The lowest-frequency component, i.e., the curve 106 (HLL) is further subjected to a thinning treatment.

How to thin the curve, in other words, how many datum are thinned in the thinning treatment may be experimentally optimized. The optimization of the thinning treatment may result in the optimization of the separation of frequency bands in the first multiresolution analysis so that a desired frequency appears in the center of a band.

In the present embodiment, 1 datum is removed from 40 data in the thinning treatment. FIG. 11 is the result of the thinning treatment of the curve 106 (HLL) in FIG. 9B. The vertical axis is a displacement scale ( $\mu\text{m}$ ) of surface profile. The lateral axis is an evaluation length scale. In the present embodiment, the evaluation length is 12 mm.

The thinned curve 106 (HLL) shown in FIG. 11 is further subjected to the second multiresolution transformation.

FIG. 9C shows 6 frequency components obtained in the second multiresolution analysis.

A curve 107 is the highest-frequency component having a frequency of from 26 to 106  $\mu\text{m}$  obtained in the second multiresolution analysis, which may be hereinafter represented as LHH.

A curve 108 is the second highest-frequency component having a frequency of from 53 to 183  $\mu\text{m}$  obtained in the second multiresolution analysis, which may be hereinafter represented as LHL.

A curve 109 is the third highest-frequency component having a frequency of from 106 to 318  $\mu\text{m}$  obtained in the second multiresolution analysis, which may be hereinafter represented as LMH.

A curve 110 is the fourth highest-frequency component having a frequency of from 214 to 551  $\mu\text{m}$  obtained in the second multiresolution analysis, which may be hereinafter represented as LML.

A curve 111 is the fifth highest-frequency component having a frequency of from 431 to 954  $\mu\text{m}$  obtained in the second multiresolution analysis, which may be hereinafter represented as LLH.

A curve 112 is the lowest-frequency component having a frequency of from 867 to 1654  $\mu\text{m}$  obtained in the second multiresolution analysis, which may be hereinafter represented as LLL.

FIG. 12 is a graph showing frequency bands separated in the second multiresolution analysis. The lateral axis represents the number of peaks and valleys per 1 mm when assuming a profile as a sine curve. The vertical axis represents the ratio of each of the frequency bands.

In FIG. 12, a curve 127 is a band of the highest-frequency component in the second multiresolution analysis. A curve 128 is a band of the second highest-frequency component in the second multiresolution analysis. A curve 129 is a band of the third highest-frequency component in the second multiresolution analysis. A curve 130 is a band of the fourth highest-frequency component in the second multiresolution analysis. A curve 131 is a band of the fifth highest-frequency component in the second multiresolution analysis. A curve 132 is a band of the lowest-frequency component in the second multiresolution analysis.

FIG. 12 indicates that when the number of peaks and valleys per 1 mm is 0.2 or less, it appears in the curve 132 only.

When the number of peaks and valleys per 1 mm is 11, it most strongly appears in the curve 128 corresponding to the curve 110 (LML) in FIG. 9C.

It depends on the frequency of a surface roughness in which curve in FIG. 9C it may appear.

In other words, relatively fine irregularities appear in the curves in the upper side of FIG. 9C while relatively coarse irregularities appear in the curves in the lower side of FIG. 9C.

Namely, a surface profile is separated into the plural curves 107 to 112 based on the frequency, as illustrated in FIG. 9C. Therefore, the number of peaks and valleys in each frequency band can be separately measured.

The curves 107 to 112 are further subjected to the calculation of the center-line average roughness Ra (i.e., WRa), maximum height, Rmax, and ten points average roughness Rz according to JIS B0601-1982. The calculated values thereof are shown in the chart (c).

The results of the above example are shown in Table 1.

TABLE 1

| Multiresolution |         | Surface Roughness (μm) |        |        |
|-----------------|---------|------------------------|--------|--------|
| Analysis        | Signals | Ra                     | Rmax   | Rz     |
| 1 <sup>st</sup> | HHH     | 0.0045                 | 0.0505 | 0.0050 |
|                 | HHL     | 0.0027                 | 0.0398 | 0.0025 |
|                 | HMH     | 0.0023                 | 0.0120 | 0.0102 |
|                 | HML     | 0.0039                 | 0.0330 | 0.0263 |
|                 | HLH     | 0.0024                 | 0.0758 | 0.0448 |
|                 | HLL     | 0.1753                 | 0.7985 | 0.6989 |
| 2 <sup>nd</sup> | LHH     | 0.0042                 | 0.0665 | 0.0045 |
|                 | LHL     | 0.0110                 | 0.1637 | 0.0121 |
|                 | LMH     | 0.0287                 | 0.0764 | 0.0680 |
|                 | LML     | 0.0620                 | 0.3000 | 0.2653 |
|                 | LLH     | 0.0462                 | 0.2606 | 0.2131 |
|                 | LLL     | 0.0888                 | 0.3737 | 0.2619 |

In the same manner as above, photoreceptors prepared in the later-described Examples and Comparative Examples are subjected to the wavelet transformation multiresolution analysis to calculate WRa of each frequency component. The photoreceptors are further subjected to a solid lubricant receptivity test described later. A relation between WRa and solid lubricant receptivity, more specifically, contributing rate of each frequency component to solid lubricant receptivity, is estimated by multivariate analysis using a statistical software program JMP Ver. 5.01a (from SAS Institute).

Roughening of a surface of a photoreceptor can be achieved by adding a material (e.g., a filler) capable of controlling surface profile to a surface layer coating liquid, controlling photoreceptor manufacturing conditions, or undergoing a mechanical treatment, for example.

Next, the electrophotographic photoreceptor of the present invention is described in detail.

FIG. 13 is a schematic view illustrating an embodiment of the photoreceptor of the present invention which includes, in order from an innermost side thereof, a conductive substrate 21, a photosensitive layer 27 including a charge generation layer 25 and a charge transport layer 26, and a surface layer 28.

FIG. 14 is a schematic view illustrating another embodiment of the photoreceptor of the present invention which includes, in order from an innermost side thereof, a conductive substrate 21, an undercoat layer 24, a photosensitive layer 27 including a charge generation layer 25 and a charge transport layer 26, and a surface layer 28.

Suitable materials for the conductive substrate 21 include material having a volume resistivity not greater than  $10^{10}$   $\Omega\cdot\text{cm}$ . Specific examples of such materials include, but are not limited to, plastic films, plastic cylinders, or paper sheets, on the surface of which a metal such as aluminum, nickel, chromium, nichrome, copper, gold, silver, platinum, and the

like, or a metal oxide such as tin oxides, indium oxides, and the like, is formed by deposition or sputtering. In addition, a metal cylinder can also be used as the conductive substrate 21, which is prepared by tubing a metal such as aluminum, aluminum alloys, nickel, and stainless steel by a method such as a drawing ironing method, an impact ironing method, an extruded ironing method, and an extruded drawing method, and then treating the surface of the tube by cutting, super finishing, polishing, and the like treatments.

10 The undercoat layer 24 may be provided between the conductive substrate 21 and the photosensitive layer 27, as illustrated in FIG. 14, for the purpose of improving adhesion and coating properties of the upper layer and preventing the occurrence of moiré and charge injection from the conductive substrate 21.

15 The undercoat layer 24 is comprised primarily of a resin. Because the photosensitive layer 27 is coated on the undercoat layer 24, the undercoat layer 24 preferably comprises a thermosetting resin that has poor solubility in organic solvents. Specific preferred examples of such resins include, but are not limited to, polyurethane resins, melamine resins, and alkyd-melamine resins. The undercoat layer 24 may be formed by coating a coating liquid in which a resin is dissolved in a solvent such as tetrahydrofuran, cyclohexane, dioxane, dichloroethane, and butanone.

20 The undercoat layer 24 may include fine particles of a metal or a metal oxide for the purpose of controlling conductivity and preventing the occurrence of moiré. Specifically, titanium oxides are preferable.

25 The fine particles may be subjected to a dispersion treatment using a ball mill, an attritor, a sand mill, or the like, with a solvent such as tetrahydrofuran, cyclohexanone, dioxane, dichloroethane, and butanone, and then mixed with a resin to prepare a coating liquid.

30 The undercoat layer 24 is formed by applying the coating liquid to the conductive substrate 21 by a dip coating method, a spray coating method, a bead coating method, or the like, upon application of heating, if needed.

35 The undercoat layer 24 generally has a thickness of from 2 to 5  $\mu\text{m}$ , and preferably less than 3  $\mu\text{m}$  to reduce residual potential.

The photosensitive layer 27 may be a multilayer including the charge generation layer 25 and the charge transport layer 26.

40 The charge generation layer 25 has a function of generating charge upon exposure to light. The charge generation layer 25 includes a charge generation material as the main component and may include a binder resin, if needed. Suitable charge generation materials include both inorganic materials and organic materials.

45 Specific examples of usable inorganic materials for the charge generation material include, but are not limited to, crystalline selenium, amorphous selenium, selenium-tellurium, selenium-tellurium-halogen, selenium-arsenic compounds, and amorphous silicon. An amorphous silicon in which dangling bonds are terminated with a hydrogen or halogen atom and an amorphous silicon doped with a boron or phosphorus atom are also preferable.

50 Specific examples of usable organic materials for the charge generation material include, but are not limited to, metal phthalocyanines such as titanyl phthalocyanine and chlorogallium phthalocyanine; metal-free phthalocyanines; azulene salt pigments; squaric acid methine pigments; symmetric or asymmetric azo pigments having a carbazole skeleton; symmetric or asymmetric azo pigments having a triphenylamine skeleton; symmetric or asymmetric azo pigments having a fluorenone skeleton; and perylene pigments.

## 17

Among these materials, metal phthalocyanines, symmetric or asymmetric azo pigments having a fluorenone skeleton, symmetric or asymmetric azo pigments having a triphenylamine skeleton, and perylene pigments are preferable because they have a high charge generation quantum efficiency. These materials can be used alone or in combination.

Specific examples of usable binder resins for the charge generation layer 25 include, but are not limited to, polyamide, polyurethane, epoxy resins, polyketone, polycarbonate, polyarylate, silicone resins, acrylic resins, polyvinyl butyral, polyvinyl formal, polyvinyl ketone, polystyrene, poly-N-vinylcarbazole, and polyacrylamide. Additionally, charge transport polymers, to be described in detail later, are also usable as the binder resin. Among these resins, polyvinyl butyral is preferable. These resins can be used alone or in combination.

The charge generation layer 25 may be formed by a vacuum method or a casting method.

The former includes a vacuum deposition method, a glow discharge decomposition method, an ion plating method, a sputtering method, a reactive sputtering method, and a CVD (chemical vapor deposition) method, for example. These methods can form a layer comprising the above-described inorganic or organic material in good condition.

In the latter, first, the above-described inorganic or organic material, optionally along with a binder resin, is dispersed in a solvent such as methyl ethyl ketone, tetrahydrofuran, cyclohexanone, dioxane, dichloroethane, and butanone, using a ball mill, an attritor, a sand mill, or the like. The resultant dispersion may be diluted as appropriate. Among these solvents, methyl ethyl ketone, tetrahydrofuran, and cyclohexanone are more preferable compared to chlorobenzene, dichloromethane, toluene, or xylene, because of being environmentally-friendly. The dispersion is coated by a dip coating method, a spray coat method, a bead coat method, or the like.

The charge generation layer 25 preferably has a thickness of from 0.01 to 5  $\mu\text{m}$ . Reduction of residual potential and increase of sensitivity may be achieved by thickening the charge generation layer 25. At the same time, deterioration of chargeability (such as charge retention ability and formation of space charge) is caused by thickening of the charge generation layer 25. To balance these properties, the charge generation layer 25 more preferably has a thickness of from 0.05 to 2  $\mu\text{m}$ .

The charge generation layer 25 may optionally include a low-molecular-weight compound such as an antioxidant, a plasticizer, a lubricant, and an ultraviolet absorber, and/or a leveling agent. These compounds can be used alone or in combination. Because too large an amount of a low-molecular-weight compound and/or a leveling agent may cause deterioration of sensitivity, the content thereof in the charge generation layer 25 is preferably from 0.1 to 20 parts by weight, more preferably from 0.1 to 10 parts by weight, and most preferably from 0.001 to 0.1 parts by weight, based on 100 parts by weight of resins.

The charge transport layer 26 has a function of transporting charges generated in the charge generation layer 25 so as to neutralize charges on the surface of the photoreceptor. The charge transport layer 26 is comprised primarily of a charge transport material and a binder resin.

## 18

Charge transport materials include low-molecular-weight electron transport materials, hole transport materials, and charge transport polymers.

Specific examples of usable electron transport materials include, but are not limited to, electron accepting materials such as asymmetric diphenoquinone derivatives, fluorene derivatives, and naphthalimide derivatives. These electron transport materials can be used alone or in combination.

Specific examples of usable hole transport materials include, but are not limited to, electron releasing materials such as oxazole derivatives, oxadiazole derivatives, imidazole derivatives, triphenylamine derivatives, butadiene derivatives, 9-(p-diethylaminostyrylanthracene), 1,1-bis(4-dibenzylaminophenyl)propane, styrylanthracene, styrylpyrazoline, phenylhydrazones,  $\alpha$ -phenylstilbene derivatives, thiazole derivatives, triazole derivatives, phenazine derivatives, acridine derivatives, benzofuran derivatives, benzimidazole derivatives, and thiophene derivatives. These hole transport materials can be used alone or in combination.

Specific examples of usable charge transport polymers include, but are not limited to, polymers having a carbazole ring such as poly-N-vinylcarbazole; polymers having a hydrazone structure described in JP-A 57-78402, the disclosure thereof being incorporated herein by reference; polysilylene polymers described in JP-A 63-285552, the disclosure thereof being incorporated herein by reference; and aromatic polycarbonates represented by the general formulae (1) to (6) in JP-A 2001-330973, the disclosure thereof being incorporated herein by reference. These charge transport polymers can be used alone or in combination. Among these compounds, aromatic polycarbonates described in JP-A 2001-330973 are preferable because of having good electrostatic properties.

Compared to low-molecular-weight charge transport materials, charge transport polymers are more advantageous because they can prevent migration of materials composing the charge transport layer 26 to the surface layer 28 such as a cross-linked resin surface layer and a thermoplastic resin surface layer, which may cause insufficient hardening of the cross-linked resin surface layer. Additionally, because charge transport polymers (i.e., high-molecular-weight charge transport materials) have excellent heat resistance, the charge transport layer 26 is unlikely to deteriorate due to hardening heat of the surface layer 28 such as a cross-linked resin surface layer and a thermoplastic resin surface layer.

Specific examples of usable binder resins for the charge transport layer 26 include, but are not limited to, thermoplastic and thermosetting resins such as polystyrene, polyester, polyvinyl, polyarylate, polycarbonate, acrylic resins, silicone resins, fluorocarbon resins, epoxy resins, melamine resins, urethane resins, phenol resins, and alkyd resins. Among these materials, polystyrene, polyester, polyarylate, and polycarbonate are preferable because of having excellent charge transportability. The charge transport layer 26 is not required to have mechanical strength because the surface layer 28 is provided thereon. Therefore, materials with high transparency and low mechanical strength, such as polystyrene, which have not been practically used, can also be used as the binder resin for the charge transport layer 26.

The above-described binder resins can be used alone or in combination. Alternatively, 2 or more monomers of the

binder resins may be copolymerized with each other, or further copolymerized with a charge transport material.

Electrically-inactive polymers that include no photoconductive chemical structure (e.g., a triarylamine structure) may be added to the charge transport layer **26** for its reformulation. For example, the following compounds are usable: Cardo polyesters having a bulky skeleton such as a fluorene skeleton; polyesters such as polyethylene terephthalate and polyethylene naphthalate; polycarbonates in which the 3,3' position of the phenol composition of a bisphenol-type polycarbonate is substituted with an alkyl group (e.g., C-type poly carbonates); polycarbonates in which a geminal methyl group of bisphenol A is substituted with a long-chain alkyl group having 2 or more carbon atoms; polycarbonates having a biphenyl or biphenyl ether skeleton; polycaprolactones; polycarbonates having a long-chain alkyl skeleton similar to a polycaprolactone, described in JP-A 07-292095, the disclosure thereof being incorporated herein by reference; acrylic resin; polystyrenes; and hydrogenated butadienes.

When the above compounds are used in combination with the binder resins, the content thereof in the charge transport layer **26** is preferably 50% or less by weight based on solid contents so as not to deteriorate sensitivity to light attenuation.

When the charge transport layer **26** includes a low-molecular-weight charge transport material, the content thereof is preferably from 40 to 200 parts by weight, more preferably from 70 to 100 parts by weight, based on 100 parts by weight of resins.

When the charge transport layer **26** includes a charge transport polymer (i.e., a high-molecular-weight charge transport material), the charge transport polymer is preferably a copolymer in which 100 parts by weight of a charge transport component and 0 to 200 parts by weight, more preferably from 80 to 150 parts by weight, of a resin component are copolymerized.

When the charge transport layer **26** includes 2 or more charge transport materials, the difference among the charge transport materials in ionization potential is preferably as small as possible. More specifically, the difference in ionization potential is preferably 0.10 eV or less. Within such a range, one charge transport material is prevented from trapping other transport materials.

Similarly, when the charge transport layer **26** includes a charge transport material and a curable charge transport material, to be described in detail later, the difference in ionization potential is preferably 0.10 eV or less.

The ionization potential of charge transport materials can be measured with an atmospheric photoemission yield spectroscopic instrument AC-1 from Riken Keiki Co., Ltd.

To achieve high sensitivity, the charge transport layer **26** preferably includes a charge transport material in an amount of 70 parts or more by weight based on 100 parts by weight of resins. In particular, monomers and dimers of  $\alpha$ -phenylstilbene compounds, benzidine compounds, and butadiene compounds, and charge transport polymers having a main chain or a side chain with the structure of the above monomers and dimers, are preferable for the charge transport material because of having high charge transportability.

Specific examples of usable solvents for coating the charge transport layer **26** include, but are not limited to, ketones (e.g., methyl ethyl ketone, acetone, methyl isobutyl ketone, cyclohexanone); ethers (e.g., dioxane, tetrahydrofuran, ethyl cellosolve); aromatic solvents (e.g., toluene, xylene); halogen-containing solvents (e.g., chlorobenzene, dichloromethane); and esters (e.g., ethyl acetate, butyl acetate).

The charge transport layer **26** may be formed by coating a coating liquid in which a mixture or a copolymer comprised primarily of a charge transport material and a binder resin is dissolved or dispersed in the above-described solvent, followed by drying. The coating liquid may be coated by a dip coating method, a spray coating method, a ring coating method, a roll coater method, a gravure coating method, a nozzle coating method, or a screen printing method, for example.

Because the surface layer **28** is provided on the charge transport layer **26**, the charge transport layer **26** may not be abraded. Therefore, it is not necessary to thicken the charge transport layer **26**.

Accordingly, the charge transport layer **26** preferably has a thickness of from 10 to 40  $\mu\text{m}$ , and more preferably from 15 to 30  $\mu\text{m}$ , to have satisfactory sensitivity and chargeability.

The charge transport layer **26** may optionally include a low-molecular-weight compound such as an antioxidant, a plasticizer, a lubricant, and an ultraviolet absorber, and/or a leveling agent. These compounds can be used alone or in combination.

Because too large an amount of a low-molecular-weight compound and/or a leveling agent may cause deterioration of sensitivity, the content thereof in the charge transport layer **26** is preferably from 0.1 to 20 parts by weight, more preferably from 0.1 to 10 parts by weight, and most preferably from 0.001 to 0.1 parts by weight, based on 100 parts by weight of resins.

Preferably, the surface layer **28** is a cross-linked resin surface layer or a thermoplastic resin surface layer.

The cross-linked resin surface layer is a layer for protecting the surface of the photoreceptor. The cross-linked resin surface layer is formed by coating a coating liquid, upon which a polycondensation reaction takes place to form a resin having a cross-linked structure. Such a resin having a cross-linked structure has high abrasion resistance.

The cross-linked resin surface layer preferably includes a cross-linked body of a cross-linkable charge transport material. Specific examples of usable cross-linkable charge transport materials include, but are not limited to, polymerizable or cross-linkable monomers and oligomers such as chain-growth-polymerizable compounds having an acryloyloxy or styrene group; and step-growth-polymerizable compounds having a hydroxyl, alkoxyisilyl, or isocyanate group. In view of electrophotographic properties, versatility, and manufacturing stability of the resultant photoreceptor, a combination of a hole transport material and a chain-growth-polymerizable compound is preferable. In particular, a cross-linked body of a compound including both a hole transport group and an acryloyloxy group is more preferable. Cross-linkable materials may be cross-linked upon application of heat, light, or radial ray. The cross-linked body preferably has a three-dimensional cross-linking structure.

Specific examples of usable polymerizable or cross-linkable materials further include compounds having a charge transport structure and 1 or more methacryloyloxy or acryloyloxy groups. Such compounds may be optionally used in combination with monomers or oligomers having no charge transport structure and 1 or more methacryloyloxy or acryloyloxy groups.

A coating liquid in which at least one compound described above is included is subjected to cross-linking and curing reactions upon application of energy such as heat, light, or radial ray such as electron beam and  $\gamma$  ray.

Preferably, the cross-linkable charge transport materials have a triarylamine structure. More preferably, the cross-linkable charge transport materials have a triarylamine structure having a monofunctional radical-polymerizable group, to cross-link with binder resins.

The following compound (A) is one preferred example for the cross-linkable charge transport material:



wherein each of d, e, and f independently represents an integer of 0 or 1; each of g and h independently represents an integer of from 0 to 3; R<sub>13</sub> represents a hydrogen atom or a methyl group; each of R<sub>14</sub> and R<sub>15</sub> independently represents an alkyl group having 1 to 6 carbon atoms, wherein multiple R<sub>14</sub> and R<sub>15</sub> may be, but need not necessarily be, the same; and Z represents a single bond, a methylene group, an ethylene group, —CH<sub>2</sub>CH<sub>2</sub>O—,

20

25



The following compounds (B) and (C) are also preferred examples for the cross-linkable charge transport material.

(2-[4'-(di-p-tolyl-amino)-biphenyl-4-yl]-ethyl acrylate)

20

25

30



35

40

45

(2-[4'-(di-p-tolyl-amino)-biphenyl-4-yl]acrylate)

The following compounds No. 1 to No. 26 are also preferred examples for the cross-linkable charge transport material.

50

(B)



55

No. 1

60



65

23



24  
-continued



No. 2

5

10

15

20

No. 3 25

30

35

40

№ 4

50

55

60

65



No 5

№ 6

25



No. 7

5

10

20

25

30

35

26



No. 9

40

6

50

55

60

65

$$\text{CH}_3$$



No. 8

45

50

55

60

65

No. 10



27



No. 11

28  
-continued



No. 14

5

10

15

20

25

88

N-12

CC=CC(=O)OCC(C)c1ccccc1Cc2ccccc2N(c3ccccc3)Cc4ccccc4

N-15



**29**  
-continued



No. 16

5

10

15

20

25

30

35

40



**30**  
-continued



No. 18

35

40

No. 17

45

50

55

60

65



No. 19

31  
-continued



32



30

35

40

No. 21 45



No. 23



**33**  
-continued



No. 24

**34**  
-continued



No. 26



No. 25

From the viewpoint of protection of the photosensitive layer 27, the cross-linked resin surface layer preferably has a thickness of from 3 to 15  $\mu\text{m}$ , and more preferably from 2 to 10  $\mu\text{m}$ . When the thickness is too small, the cross-linked resin surface layer may not protect the photosensitive layer 27 from mechanical abrasion applied from contacting members and electric discharge from a closely-disposed charger. Moreover, because such a thin layer is hard to level, an irregular surface with a texture like an orange peel may be produced. By contrast, when the thickness is too large, reproducibility of image may decrease due to the occurrence of charge diffusion. Additionally, when the thickness of the cross-linked resin surface layer is greater than that of the charge transport layer 26, bright section potential is likely to increase, which is not preferable.

In consideration of a case in which the surface of a photoreceptor has plural convexities and the thickness of the layer cannot be determined unambiguously, the thickness of the layer may be measured with a film thickness meter using the eddy current FISHERSCOPE® MMS® (from Fischer Instruments K.K.). The measurement may be performed at 4 or more points on a photoreceptor in the axial direction, and the measured values are averaged.

The cross-linked resin surface layer preferably includes the above-described cross-linkable charge transport material (A) in an amount of from 50 to 60% by weight. When the amount is too small, charge transportability may be poor and electric properties may deteriorate with repeated use, causing deterioration of sensitivity and increase of residual potential. When the amount is too large, the cross-linking density may decrease, resulting in poor abrasion resistance.

To more improve abrasion resistance, the cross-linked resin surface layer preferably includes a cross-linked body of a radical-polymerizable monomer having 3 or more radical-polymerizable functional groups, such as a cross-linked body of a trimethylolpropane triacrylate having 3 radical-polymerizable functional groups, as a binder material.

As another example, a cross-linked body of a caprolactone-modified dipentaerythritol hexaacrylate or a dipentaerythritol hexaacrylate may also be included in the cross-linked resin

surface layer as the cross-linked body of a radical-polymerizable monomer having 3 or more radical-polymerizable functional groups. These materials may improve abrasion resistance and toughness of the layer.

The cross-linked resin surface layer preferably includes a cross-linked body of a trimethylolpropane triacrylate in an amount of 10% by weight or more and less than 50% by weight. When the amount is too small, the cross-linking density may be too low, resulting in poor mechanical strength. When the amount is too large, electric properties may be poor.

Specific examples of usable radical-polymerizable monomers having 3 or more functional groups which have no charge transport structure include, but are not limited to, trimethylolpropane triacrylate, caprolactone-modified dipentaerythritol hexaacrylate, and dipentaerythritol hexaacrylate.

These materials are available from Tokyo Chemical Industry Co., Ltd., or Nippon Kayaku Co., Ltd. under the trade name of KAYARD DPCA series and KAYARD DPNA series.

To accelerate or stabilize curing, an initiator such as IRGACURE® 184 (from Ciba) in an amount of from 5 to 10% by weight (based on solid contents) may be added to the cross-linked resin surface layer.

The cross-linked resin surface layer is preferably formed by coating and curing a coating liquid comprising a cross-linkable charge transport material, a trimethylolpropane triacrylate, a cross-linkable silicone material, and a non-cross-linkable silicone material on the photosensitive layer 27.

Specific examples of usable solvents for preparing the coating liquid for the cross-linked resin surface layer include, but are not limited to, ethers (e.g., dioxane, tetrahydrofuran, ethyl cellosolve); aromatic solvents (e.g., toluene, xylene); halogen-containing solvents (e.g., chlorobenzene, dichloromethane); esters (e.g., ethyl acetate, butyl acetate); cellosolves (e.g., ethoxyethanol); and propylene glycols (e.g., 1-methoxy-2-propanol). In particular, methyl ethyl ketone, tetrahydrofuran, cyclohexanone, and 1-methoxy-2-propanol are more preferable compared to chlorobenzene, dichloromethane, toluene, or xylene, because of being environmentally-friendly. These solvents can be used alone or in combination.

The coating liquid of the cross-linked resin surface layer may be coated by a dip coating method, a spray coating method, a ring coating method, a roll coater method, a gravure coating method, a nozzle coating method, or a screen printing method, for example. Because coating liquids generally have a relatively short pot life, methods capable of coating with a small amount of a coating liquid are advantages from the viewpoint of environmental consciousness and cost. Among the above coating methods, a spray coating method and a ring coating method are preferable.

When forming the cross-linked resin surface layer, UV emitting light sources having the emission wavelength in the ultraviolet region, such as high-pressure mercury lamps and metal halide lamps, are usable. Additionally, visible light emitting light sources are also usable, depending on the absorption wavelength of radical-polymerizable compounds, photopolymerization initiators, etc. The amount of emission light is preferably from 50 to 1,000 mW/cm<sup>2</sup>. When the amount emission light is too small, it takes too long a time for the curing reaction. When the amount of emission light is too large, the curing reaction may proceed unevenly, generating local wrinkles on the cross-linked resin surface layer and/or a lot of residual groups which have not been reacted and terminal ends which have lost reactivity. Additionally, the cross-linking reaction may proceed so quickly that the inner stress may increase, thereby causing cracks and peeling of the layer.

The cross-linked resin surface layer may optionally include a low-molecular-weight compound such as an antioxidant, a plasticizer, a lubricant, and an ultraviolet absorber, and/or a leveling agent. Also, the cross-linked resin surface layer may optionally include the above-described polymer compounds usable for the charge transport layer 26. These compounds can be used alone or in combination. Because too large an amount of a low-molecular-weight compound and/or a leveling agent may cause deterioration of sensitivity, the content thereof in the cross-linked resin surface layer is preferably from 0.1 to 20% by weight, and more preferably from 0.1 to 10% by weight. In particular, the content of a leveling agent is preferably from 0.1 to 5% by weight.

As described above, the surface layer 28 may be a thermoplastic resin surface layer. The thermoplastic resin surface layer is a layer for protecting the surface of the photoreceptor.

The thermoplastic resin surface layer is preferably formed by coating a coating liquid comprising a charge transport material, a thermoplastic resin, a cross-linkable silicone material, and a non-cross-linkable silicone material on the photosensitive layer 27. The coating liquid is subjected to a cross-linking reaction so that the cross-linkable silicone material is moderately polymerized.

The charge transport materials and thermoplastic resins usable for the charge transport layer 26 are also usable for the thermoplastic resin surface layer.

The thermoplastic resin surface layer preferably has a thickness of from 3 to 15 µm. The lower limit depends on the balance between manufacturing cost and effectiveness of the layer. The upper limit depends on the homogeneity between electrostatic properties (e.g., charge stability, light attenuation sensitivity) and quality of the layer.

In consideration of a case in which the surface of a photoreceptor has plural convexities and the thickness of the layer cannot be determined unambiguously, the thickness of the layer may be measured with a film thickness meter using the eddy current FISHERSCOPE® MMS® (from Fischer Instruments K.K.). The measurement may be performed at 4 or more points on a photoreceptor in the axial direction, and the measured values are averaged.

When moderately curing the cross-linkable silicone material in the thermoplastic resin surface layer, UV emitting light sources having the emission wavelength in the ultraviolet region, such as high-pressure mercury lamps and metal halide lamps, are usable. Additionally, visible light emitting light sources are also usable, depending on the absorption wavelength of radical-polymerizable compounds, photopolymerization initiators, etc. The amount of emission light is preferably from 50 to 1,000 mW/cm<sup>2</sup>. When the amount emission light is too small, it takes too long a time for the curing reaction. When the amount of emission light is too large, the curing reaction may proceed unevenly, degrading the charge transport material and electric properties.

The surface of the photoreceptor can be roughened by adding a cross-linkable silicone material and a non-cross-linkable material to the surface layer 28.

In order to satisfy the inequations (i) to (v), the surface of the photoreceptor may be roughened. One specific method of roughening the surface of the photoreceptor includes adding materials capable of controlling surface profile to the surface layer 28.

Specific examples of such materials include fillers, zol-gel coating materials, polymer blends comprising various resins with different glass transition points, organic fine particles, foaming agents, and a large amount of silicone oil.

Another specific method includes controlling layer forming conditions by adding a large amount of water or liquid materials having different boiling points to the coating liquid of the surface layer **28**.

Another specific method includes spraying an organic solvent or water on a wet layer that is formed immediately after coating the coating liquid and is not yet subjected to curing.

Alternatively, the surface layer **28** may be subjected to a sandblast treatment or a surface abrasion treatment using an abrasion paper such as a lapping film after curing.

The above-described methods can be combined, if needed. In the present embodiment, the inequations (i) to (v) are achieved by adding both a cross-linkable silicone material and a non-cross-linkable silicone material to the coating liquid of the surface layer **28**. If a cross-linkable silicone material or a non-cross-linkable silicone material is solely added to the coating liquid, the inequations (i) to (v) may not be achieved.

The cross-linkable silicone material may be, for example, a reactive silicone material in which at least one terminal of a polysiloxane is methacrylate-modified. By adding such a cross-linkable silicone material in the coating liquid of the surface layer **28**, the inequation (ii) representing a surface profile at LHH frequency is satisfied. The content of the cross-linkable silicone material in the coating liquid is preferably from 1 to 5% by weight based on solid contents. Such cross-linkable silicone materials may be available from, for example, Shin-Etsu Chemical Co., Ltd. under the trade name of X-22 series.

The non-cross-linkable silicone material may be, for example, a straight-chain polymer comprised of siloxane bonds, more specifically, a phenyl-modified methylphenyl silicone oil in which a part of side chains of a polysiloxane are phenyl groups. By adding such a non-cross-linkable silicone material in the coating liquid of the surface layer **28**, the inequation (i) representing a surface profile at LMH frequency is satisfied. The content of the non-cross-linkable silicone material in the coating liquid is preferably from 1 to 5% by weight based on solid contents. Such non-cross-linkable silicone materials may be available from, for example, Shin-Etsu Chemical Co., Ltd. under the trade name of KF series.

Next, the image forming apparatus of the present invention is described in detail. The image forming apparatus of the present invention comprises an image forming unit and a lubricant applicator. For the sake of simplicity, the image forming unit and the lubricant applicator will be described separately.

First, exemplary embodiments of the image forming unit are described in detail.

For the sake of simplicity, the same reference number will be given to identical constituent elements such as parts and materials having the same functions and redundant descriptions thereof omitted unless otherwise stated.

FIG. 15 is a schematic view illustrating an embodiment of the image forming unit.

A photoreceptor **11** is the photoreceptor of the present invention having the above-described surface layer. The photoreceptor **11** is in the form of a drum in FIG. 15. Alternatively, the photoreceptor **11** may be in the form of a sheet or an endless belt.

A charger **12** may be a corotron, a scorotron, a solid state charger, or a charging roller, for example. From the viewpoint of consumption energy saving, the charger **12** is preferably provided in contact with or proximally to the photoreceptor **11**. To prevent contamination of the charger **12**, it is more preferable to provide the charger **12** proximally to the photo-

receptor **11** so that a reasonable gap is formed between the photoreceptor **11** and the charger **12**.

A transferrer **16** may also be a corotron, a scorotron, a solid state charger, or a charging roller, for example. Preferably, the transferrer **16** may be a combination of a transfer charger and a separation charger.

An irradiator **13** and a neutralizer **1A** each may be a light source such as a fluorescent lamp, a tungsten lamp, a halogen lamp, a mercury lamp, a sodium lamp, a light-emitting diode (LED), a laser diode (LD), and an electroluminescence (EL). To emit light having a desired wavelength, these light sources can be used with a filter such as a sharp cut filter, a bandpass filter, a near-infrared cut filter, a dichroic filter, an interference filter, and a color temperature conversion filter.

A developing device **14** develops a latent image on the photoreceptor **11** with a toner **15**. The toner **15** is transferred from the photoreceptor **11** onto a recording medium **18** such as a printing paper and an OHP sheet. The toner **15** is then fixed on the recording medium **18** in a fixing device **19**. Some toner particles may remain on the photoreceptor **11** without being transferred onto the recording medium **18**. Such residual toner particles are removed from the photoreceptor **11** with a cleaner **17**. The cleaner **17** may be, for example, a rubber blade, a fur brush, or a magnetic fur brush.

When the photoreceptor **11** is positively (or negatively) charged and irradiated with light containing image information, a positive (or negative) electrostatic latent image is formed thereon. When the positive (or negative) electrostatic latent image is developed with a negatively-charged (or positively-charged) toner, a positive image is obtained. By contrast, when the positive (or negative) electrostatic latent image is developed with a positively-charged (or negatively-charged) toner, a negative image is obtained.

FIG. 16 is a schematic view illustrating another embodiment of the image forming unit.

A photoreceptor **11** is the photoreceptor of the present invention having the above-described surface layer. The photoreceptor **11** is in the form of a belt in FIG. 16. Alternatively, the photoreceptor **11** may be in the form of a drum or an endless belt.

The photoreceptor **11** is driven by driving members **1C** and repeatedly subjected to the processes of charging with a charger **12**, image irradiation with an image irradiator **13**, development with a developing device (not shown), transfer with a transferrer **16**, pre-cleaning irradiation with a pre-cleaning irradiator **1B**, cleaning with a cleaner **17**, and neutralization with a neutralizer **1A**. In FIG. 16, the pre-cleaning irradiator **1B** irradiates the photoreceptor **11** from the substrate side thereof because the substrate is transparent in this embodiment.

Alternatively, the pre-cleaning irradiator **1B** may irradiate the photoreceptor **11** from the photosensitive layer side thereof. Similarly, the image irradiator **13** and the neutralizer **1A** each may irradiate the photoreceptor **11** from the substrate side thereof.

In addition to the image irradiator **13**, the pre-cleaning irradiator **1B**, and the neutralizer **1A**, other members that irradiate the photoreceptor **11** with light, such as a pre-transfer irradiator and a pre-image irradiation irradiator, may be provided.

The above-described image forming unit is mountable on image forming apparatuses such as copiers, facsimile machines, and printers. Alternatively, the image forming unit may compose a process cartridge that is mountable on image forming apparatuses. FIG. 17 is a schematic view illustrating an embodiment of the process cartridge of the present invention. A photoreceptor **11** is the photoreceptor of the present

invention having the above-described surface layer. The photoreceptor **11** is in the form of a drum in FIG. 17. Alternatively, the photoreceptor **11** may be in the form of a sheet or an endless belt.

FIG. 18 is a schematic view illustrating another embodiment of the image forming unit.

Around a photoreceptor **11**, a charger **12**, an irradiator **13**, a black developing device **14Bk**, a cyan developing device **14C**, a magenta developing device **14M**, a yellow developing device **14Y**, an intermediate transfer belt **1F**, and a cleaner **17** are provided in this order. The additional characters Bk, C, M, and Y representing toner colors of black, cyan, magenta, and yellow, respectively, may be added or omitted as appropriate.

The photoreceptor **11** is the photoreceptor of the present invention having the above-described surface layer. The developing devices **14Bk**, **14C**, **14M**, and **14Y** are independently controllable.

A first transerrer **1D** transfers a toner image formed on the photoreceptor **11** onto the intermediate transfer belt **1F**. The first transerrer **1D** is provided inside the intermediate transfer belt **1F**, and is movable so that the intermediate transfer belt **1F** contacts with/separates from the photoreceptor **11**. The intermediate transfer belt **1F** is brought into contact with the photoreceptor **11** only during a toner image is transferred from the photoreceptor **11** onto the intermediate transfer belt **1F**.

Each color toner image is sequentially formed and superimposed on one another on the intermediate transfer belt **1F** to form a composite toner image. A second transerrer **1E** transfers the composite toner image from the intermediate transfer belt **1F** onto a recording medium **18**. The composite toner image is fixed on the recording medium **18** in a fixing device **19**. The second transerrer **1E** is movable so as to contact with/separate from the intermediate transfer belt **1F**. The second transerrer **1E** is brought into contact with the intermediate transfer belt **1F** only during the transfer of toner image.

A conventional image forming unit employing an intermediate transfer drum has a disadvantage that thick paper is not usable as the recording medium. This is because the recording medium is required to be flexible so as to be electrostatically adsorbed to the drum and each color toner image is superimposed one another directly on the recording medium.

By contrast, in the image forming unit illustrated in FIG. 18 employing the intermediate transfer belt **1F** has an advantage that usable recording medium are not limited to any particular material. This is because each color toner image is superimposed one another on the intermediate transfer belt **1F**.

FIG. 19 is a schematic view illustrating another embodiment of the image forming unit. The image forming unit includes photoreceptors **11Y**, **11M**, **11C**, and **11Bk**. Each of the photoreceptors **11Y**, **11M**, **11C**, and **11Bk** is the photoreceptor of the present invention having the above-described surface layer. Around the photoreceptor **11Y**, a charger **12Y**, an irradiator **13Y**, a developing device **14Y**, and a cleaner **17Y** are provided. The same are provided around the photoreceptors **11M**, **11C**, and **11Bk** as well. A conveyance transfer belt **1G** is stretched taut between driving members **1C** and contacts the photoreceptors **11Y**, **11M**, **11C**, and **11Bk** arranged in line. Transferrers **16Y**, **16M**, **16C**, and **16Bk** are provided on the opposite sides of the photoreceptors **11Y**, **11M**, **11C**, and **11Bk**, respectively, relative to the conveyance transfer belt **1G**.

The image forming unit illustrated in FIG. 19 is what is called a tandem image forming unit in which yellow, magenta, cyan, and black toner images are formed on the respective photoreceptors **11Y**, **11M**, **11C**, and **11Bk** and are sequentially transferred onto a recording medium **18** on the

conveyance transfer belt **1G**. Such a tandem image forming unit is capable of printing full-color images at higher speeds compared to an image forming unit including only one photoreceptor.

FIG. 20 is a schematic view illustrating another embodiment of the image forming unit. The image forming unit illustrated in FIG. 20 is a tandem image forming unit which employs an intermediate transfer belt **1F**.

Next, exemplary embodiments of the lubricant applicator are described in detail.

FIG. 21 is a schematic view illustrating an embodiment of the solid lubricant applicator. A lubricant applicator **3C** includes a fur brush **3B**, a solid lubricant **3A**, and a pressing spring **3E** for pressing the solid lubricant **3A** against the fur brush **3B**. The solid lubricant **3A** is compressed into a bar. The tips of the brush fibers of the fur brush **3B** are in contact with the photoreceptor **11**. The solid lubricant **3A** is drawn up on the fur brush **3B** and is conveyed to the contact point of the fur brush **3B** with the photoreceptor **11** by rotation of the fur brush **3B**. Thus, the solid lubricant **3A** is applied to the photoreceptor **11**.

The pressing spring **3E** presses the solid lubricant **3A** against the fur brush **3B** at a predetermined pressure so that the solid lubricant **3A** is constantly in contact with the fur brush **3B** even when the solid lubricant **3A** is abraded and reduced in volume with time.

In order to improve fixability of the solid lubricant **3A** on the photoreceptor **11**, a lubricant fixer may be provided. The lubricant fixer may be, for example, a blade **35** that is provided in contact with the photoreceptor **11** so as to trail the photoreceptor **11**. Alternatively, the blade **35** may be provided in contact with the photoreceptor **11** so as to face in the direction of rotation of the photoreceptor **11**.

Specific examples of usable materials for the solid lubricant **3A** include, but are not limited to, fatty acid metal salts such as lead oleate, zinc oleate, copper oleate, zinc stearate, cobalt stearate, iron stearate, copper stearate, zinc palmitate, copper palmitate, and zinc linolenate; and fluorine-containing resins such as polytetrafluoroethylene, polychlorotrifluoroethylene, polyvinylidene fluoride, polytrifluorochloroethylene, dichlorodifluoroethylene, tetrafluoroethylene-ethylene copolymer, and tetrafluoroethylene-oxafluoropropylene copolymer. Among these materials, metal salts of stearic acids, more specifically, zinc stearate is most preferable because of effectively reducing the friction coefficient of the photoreceptor **11**.

The photoreceptor **11** is the photoreceptor of the present invention having the surface layer having a specific surface profile. Therefore, the solid lubricant **3A** can be effectively applied to the surface of the photoreceptor **11**. Accordingly, the photoreceptor of the present invention expresses excellent cleanability of spherical toners.

Having generally described this invention, further understanding can be obtained by reference to certain specific examples which are provided herein for the purpose of illustration only and are not intended to be limiting. In the descriptions in the following examples, the numbers represent weight ratios in parts, unless otherwise specified.

## EXAMPLES

First, the procedures for evaluation of the below-prepared photoreceptors are described.

### (1) Measurement of Surface Profile

A photoreceptor is set to a pickup (E-DT-S02A) and subjected to a measurement using a surface texture and contour measuring instrument SURFCOM 1400D (from Tokyo

41

Seimitsu Co., Ltd.) to obtain text data of a cross-sectional curve of a surface of the photoreceptor. The evaluation length is 12 mm, the measuring speed is 0.06 mm/s, and the sampling length is 0.39  $\mu\text{m}$ .

The text data is subjected to wavelet transformation multiresolution analysis so as to be separated into 6 frequency components each having a cycle length ( $\mu\text{m}$ ) of 0 to 3, 1 to 6, 2 to 13, 4 to 25, 10 to 50, and 24 to 99.

A one-dimensional data array of the lowest frequency component having a cycle length of from 24 to 99 ( $\mu\text{m}$ ) is thinned so that the number of data array is reduced to  $\frac{1}{40}$ . The thinned one-dimensional data array is subjected to wavelet transformation multiresolution analysis so as to be separated into the 6 frequency components (LHH, LHL, LMH, LML, LLH, and LLL) each having a cycle length ( $\mu\text{m}$ ) of 26 to 106, 53 to 183, 106 to 318, 214 to 551, 431 to 954, and 867 to 1,654, respectively.

Randomly selected 4 points on each photoreceptor are subjected to the above measurement. Each text data of a cross-sectional curve is subjected to wavelet transformation and multiresolution analysis, and WR<sub>A</sub> ( $\mu\text{m}$ ) is calculated and averaged. The mother wavelet function is Harr function.

#### (2) Solid Lubricant Receptivity Test

A photoreceptor is mounted on a color printer IPSIO SP C811 (from Ricoh Co., Ltd.) to be subjected to a solid lubricant receptivity test. As the solid lubricant, zinc stearate is used. The color copier is partially modified so as to have a configuration illustrated in FIG. 22.

To keep the test conditions constant, a zinc stearate bar (i.e., a solid lubricant), an application brush, and an application blade are provided to a photoreceptor-developing device composite unit (hereinafter "PD unit"). To uniformly impregnate the zinc stearate to the application brush in advance, the PD unit is mounted on the color copier and idled for 30 minutes. The developer contained in the PD unit is completely removed.

Before mounting on the PD unit, a photoreceptor is subjected to surface observation with a laser microscope (VK-8500 from Keyence Corporation). After mounting the photoreceptor on the PD unit, the PD unit is mounted on the color copier and idled for 15 seconds. The photoreceptor is taken out of the PD unit and is subjected to the surface observation again to obtain an image of the surface.

The image is subjected to an image analysis so that domains of zinc stearate remaining on the photoreceptor are distinguished and the size and the area occupancy of the domains are calculated with MEASURE and COUNT commands of an image analysis software program IMAGE PRO PLUS Ver 3.0 (from Media Cybernetics, Inc.). An example result of the image analysis is shown in FIG. 23. The solid lubricant receptivity is evaluated with the area occupancy of the domains of zinc stearate remaining on the photoreceptor after the 15-second idling.

#### (3) Image Evaluation

A halftone pattern with a pixel density of 600 dpi  $\times$  600 dpi in which 4 dots  $\times$  4 dots are formed on an 8  $\times$  8 matrix and a blank pattern are alternately and independently produced on continuous 5 sheets of paper each. The blank pattern is visually observed to determine whether background is contaminated or not. The results are graded in the following 5 levels.

42

- 5: Very clean.
- 4: Clean.
- 3: No problem.
- 2: Slightly contaminated but no problem in practical use.
- 1: Contaminated.

#### Example 1

On each of an aluminum cylinder having a thickness of 0.8 mm, a length of 340 mm, and an outer diameter of 40 mm, and another aluminum cylinder having a thickness of 0.8 mm, a length of 340 mm, and an outer diameter of 30 mm, a undercoat layer coating liquid, a charge generation layer coating liquid, and a charge transport layer coating liquid are sequentially coated and dried in this order. Thus, an undercoat layer, a charge generation layer, and a charge transport layer having a thickness of 3.5  $\mu\text{m}$ , 0.2  $\mu\text{m}$ , and 24  $\mu\text{m}$ , respectively, are formed on each of the aluminum cylinders.

Further, a cross-linked resin surface layer coating liquid is spray-coated on the aluminum cylinders having the undercoat layer, the charge generation layer, and the charge transport layer thereon, followed by drying for 10 minutes. The aluminum cylinders are put 120 mm away from a UV curing lamp so that the cross-linked resin surface layer coating liquid is subjected to UV curing while rotating. The illuminance at that position is 550 mW/cm<sup>2</sup> when measured with an accumulated UV meter UIT-150 from Ushio Inc. The aluminum cylinders rotate at a revolution of 25 rpm. The aluminum cylinders are exposed to UV ray for 4 minutes while circulating water having a temperature of 30° C. therein, followed by drying for 30 minutes at 130° C. Thus, photoreceptors having a cross-linked resin surface layer having a thickness of 6  $\mu\text{m}$  are prepared.

The compositions of the coating layers are shown in Tables 2 to 5.

TABLE 2

| Composition of Undercoat Layer Coating Liquid |                                                 |                |
|-----------------------------------------------|-------------------------------------------------|----------------|
| Components                                    | Trade Name or Chemical Formula                  | Amount (parts) |
| Alykyd resin solution                         | BECKOLITE M6401-50 (from DIC Corporation)       | 12             |
| Melamine resin solution                       | SUPER BECKAMINE G-821-60 (from DIC Corporation) | 8.0            |
| Titanium oxide                                | CR-EL (from Ishihara Sangyo Kaisha, Ltd.)       | 40             |
| Methyl ethyl ketone                           | —                                               | 200            |

TABLE 3

| Composition of Charge Generation Layer Coating Liquid |                                | Amount<br>(parts) |
|-------------------------------------------------------|--------------------------------|-------------------|
| Components                                            | Trade Name or Chemical Formula |                   |
| Bisazo pigment                                        |                                | 5.0               |
|                                                       | (from Ricoh Co., Ltd.)         |                   |
| Polyvinyl butyral                                     | XYHL (from UCC)                | 1                 |
| Cyclohexanone                                         | —                              | 200               |
| Methyl ethyl ketone                                   | —                              | 80                |

TABLE 4

| Composition of Charge Transport Layer Coating Liquid |                                                | Amount<br>(parts) |
|------------------------------------------------------|------------------------------------------------|-------------------|
| Components                                           | Trade Name or Chemical Formula                 |                   |
| Z-type Polycarbonate                                 | PANLITE ® TS-2050 (from Teijin Chemicals Ltd.) | 10                |
| Low-molecular-weight charge transport material       |                                                | 7.0               |
| Tetrahydrofuran                                      | —                                              | 100               |
| Silicone oil (in 1% THF solution)                    | KF50-100CS (from Shin-Etsu Chemical Co., Ltd.) | 1                 |

TABLE 5

| Components                                                                                                                                   | Trade Name or Chemical Formula                  | Amount (parts) |
|----------------------------------------------------------------------------------------------------------------------------------------------|-------------------------------------------------|----------------|
| Cross-linkable charge transport material                                                                                                     |                                                 | 6.0            |
| Trimethylolpropane triacrylate                                                                                                               | KAYARAD TMPTA (from Nippon Kayaku Co., Ltd.)    | 3.0            |
| 50% THF solution of caprolactone-modified dipentaerythritol hexaacrylate                                                                     | KAYARAD DPCA-120 (from Nippon Kayaku Co., Ltd.) | 6.0            |
| 5% THF solution of a mixture of polyester-modified polydimethylsiloxane having acryl group and propoxy-modified 2-neopentylglycol diacrylate | BYK-UV3571 (from BYK Japan KK)                  | 0.24           |
| 1-Hydroxycyclohexyl phenyl ketone<br>Tris(2,4-di-tert-butylphenyl) phosphate                                                                 | IRGACURE ® 184 (from Ciba)<br>—                 | 0.60<br>0.12   |
| Tetrahydrofuran                                                                                                                              | —                                               | 68.92          |
| Cross-linkable silicone oil material                                                                                                         | X-22-174DX (from Shin-Etsu Chemical Co., Ltd.)  | 0.45           |
| Non-cross-linkable silicone oil material                                                                                                     | KF-50-100CS (from Shin-Etsu Chemical Co., Ltd.) | 0.15           |

### Example 2

The procedure in Example 1 is repeated except for changing the amount of the cross-Linkable silicone oil material to 0.75 parts.

### Example 3

The procedure in Example 1 is repeated except for changing the amount of the non-cross-linkable silicone oil material to 0.45 parts. 50

### Example 4

The procedure in Example 1 is repeated except for changing the amounts of the cross-linkable silicone oil material and the non-cross-linkable silicone oil material to 0.75 parts and 0.45 parts, respectively.

### Example 5

The procedure in Example 1 is repeated except for changing the amounts of the cross-linkable silicone oil material and the non-cross-linkable silicone oil material to 0.15 parts and 0.75 parts, respectively.

### Example 6

The procedure in Example 1 is repeated except for changing the amounts of the cross-linkable silicone oil material and the non-cross-linkable silicone oil material to 0.45 parts and 0.75 parts, respectively.

### Example 7

The procedure in Example 1 is repeated except for changing the amounts of the cross-linkable silicone oil material and the non-cross-linkable silicone oil material to 0.75 parts and 0.75 parts, respectively.

60

### Comparative Example 1

The procedure in Example 1 is repeated except for replacing the cross-linked resin surface layer coating liquid with another cross-linked resin surface layer coating liquid having the composition shown in Table 6.

TABLE 6

| Composition of Cross-linked Resin Surface Layer Coating Liquid                                                                               |                                                 |                   |
|----------------------------------------------------------------------------------------------------------------------------------------------|-------------------------------------------------|-------------------|
| Components                                                                                                                                   | Trade Name or Chemical Formula                  | Amount<br>(parts) |
| Cross-linkable charge transport material                                                                                                     |                                                 | 6.0               |
| Trimethylolpropane triacrylate                                                                                                               | KAYARAD TMPTA (from Nippon Kayaku Co., Ltd.)    | 3.0               |
| 50% THF solution of caprolactone-modified dipentaerythritol hexaacrylate                                                                     | KAYARAD DPCA-120 (from Nippon Kayaku Co., Ltd.) | 6.0               |
| 5% THF solution of a mixture of polyester-modified polydimethylsiloxane having acryl group and propoxy-modified 2-neopentylglycol diacrylate | BYK-UV3571 (from BYK Japan KK)                  | 0.24              |
| 1-Hydroxycyclohexyl phenyl ketone                                                                                                            | IRGACURE ® 184 (from Ciba)                      | 0.60              |
| Tris(2,4-di-tert-butylphenyl)phosphate                                                                                                       | —                                               | 0.12              |
| Tetrahydrofuran                                                                                                                              |                                                 | 68.92             |

## Comparative Example 2

The procedure in Example 1 is repeated except for replacing the cross-linked resin surface layer coating liquid with another cross-linked resin surface layer coating liquid having the composition shown in Table 7. 35

TABLE 7

| Composition of Cross-linked Resin Surface Layer Coating Liquid                                                                               |                                                 |                   |
|----------------------------------------------------------------------------------------------------------------------------------------------|-------------------------------------------------|-------------------|
| Components                                                                                                                                   | Trade Name or Chemical Formula                  | Amount<br>(parts) |
| Cross-linkable charge transport material                                                                                                     |                                                 | 6.0               |
| Trimethylolpropane triacrylate                                                                                                               | KAYARAD TMPTA (from Nippon Kayaku Co., Ltd.)    | 3.0               |
| 50% THF solution of caprolactone-modified dipentaerythritol hexaacrylate                                                                     | KAYARAD DPCA-120 (from Nippon Kayaku Co., Ltd.) | 6.0               |
| 5% THF solution of a mixture of polyester-modified polydimethylsiloxane having acryl group and propoxy-modified 2-neopentylglycol diacrylate | BYK-UV3571 (from BYK Japan KK)                  | 0.24              |

TABLE 7-continued

| Composition of Cross-linked Resin Surface Layer Coating Liquid |                                                                                            |                |
|----------------------------------------------------------------|--------------------------------------------------------------------------------------------|----------------|
| Components                                                     | Trade Name or Chemical Formula                                                             | Amount (parts) |
| 1-Hydroxycyclohexyl phenyl ketone                              | IRGACURE ® 184 (from Ciba)                                                                 | 0.60           |
| Tris(2,4-di-tert-butylphenyl) phosphate                        | —                                                                                          | 0.12           |
| Filler                                                         | EPOSTAR S6 (from Nippon Shokubai Co., Ltd., having average diameter of 0.3 $\mu\text{m}$ ) | 0.67           |
| Tetrahydrofuran                                                |                                                                                            | 68.9           |

## Comparative Example 3

15

## Comparative Example 7

The procedure in Comparative Example 2 is repeated except for changing the amount of the filler to 1.4 parts.

## Comparative Example 4

20

The procedure in Comparative Example 2 is repeated except for changing the amount of the filler to 3.2 parts.

## Comparative Example 5

25

The procedure in Example 1 is repeated except for replacing the cross-linked resin surface layer coating liquid with a reinforced surface layer coating liquid having the composition shown in Table 8.

The procedure in Example 1 is repeated except for changing the amounts of the cross-linkable silicone oil material and the non-cross-linkable silicone oil material to 0.75 parts and 0 part, respectively.

Each of the photoreceptors prepared in Examples 1 to 7 and Comparative Examples 1 to 7 each having a diameter of 40 mm is mounted on a yellow development station of an image forming apparatus IPSIO SP C811 (from Ricoh Co., Ltd.) to be subjected to the solid lubricant receptivity test. The linear speed of the photoreceptor is 205 mm/s. The zinc stearate and spring, which are genuine parts of the image forming apparatus, are used without modification.

The photoreceptor-developing device composite unit (i.e., PD unit) is also a genuine part. The voltage applied to the

TABLE 8

| Composition of Reinforced Surface Layer Coating Liquid |                                                                                     |                |
|--------------------------------------------------------|-------------------------------------------------------------------------------------|----------------|
| Components                                             | Trade Name or Chemical Formula                                                      | Amount (parts) |
| Z-type Polycarbonate                                   | PANLITE ® TS-2050 (from Teijin Chemicals Ltd.)                                      | 10             |
| Low-molecular-weight charge transport material         |  | 7.0            |
| $\alpha$ -Alumina                                      | SUMICORUNDUM AA-03 (from Sumitomo Chemical Co., Ltd.)                               | 5.7            |
| Disperser                                              | BYK-P104 (from BYK Japan KK)                                                        | 0.014          |
| Tetrahydrofuran                                        | —                                                                                   | 280            |
| Cyclohexanone                                          | —                                                                                   | 80             |

## Comparative Example 6

60

The procedure in Example 1 is repeated except for changing the amounts of the cross-linkable silicone oil material and the non-cross-linkable silicone oil material to 0 part and 0.75 parts, respectively.

charging roller includes an AC component having a peak-to-peak voltage of 1.5 kV and a frequency of 0.9 kHz and a DC component including a bias which charges the photoreceptor to -700 V at the beginning of the test. This charging condition is maintained throughout the test. No neutralization device is provided to the image forming apparatus.

Next, each of the photoreceptors prepared in Examples 1 to 7 and Comparative Examples 1 to 7 each having a diameter of 40 mm is mounted on a black development station of an image forming apparatus IPSIO SP C811 (from Ricoh Co., Ltd.). A printing job in which a halftone pattern with a pixel density of 600 dpi×600 dpi in which 4 dots×4 dots are formed on an 8×8 matrix and a blank pattern are alternately and independently produced on continuous 5 sheets of paper each is repeatedly executed, so that 50,000 sheets are produced in total. The paper is MY PAPER A4 (from NBS Ricoh) and the toner and developer are genuine parts of the image forming apparatus. The toner is a polymerization toner.

The photoreceptor unit is a genuine part. The voltage applied to the charging roller includes an AC component having a peak-to-peak voltage of 1.5 kV and a frequency of 0.9 kHz and a DC component including a bias which charges the photoreceptor to -700 V at the beginning of the test. This charging condition is maintained throughout the test. No neutralization device is provided to the image forming apparatus. The cleaning unit, which is a genuine part, is replaced with an unused one at every 50,000 sheets. After the test, a color test chart is produced on a PPC paper TYPE 6200A3. The test is performed at 25° C., 55% RH.

The measurement results of WRa in Examples 1 to 7 and Comparative Examples 1 to 7 are shown in FIGS. 24 to 37. The results of WRa's, the solid lubricant receptivity test, and the image evaluation in Examples 1 to 7 and Comparative Examples 1 to 7 are shown in Table 9.

TABLE 9

|                       | Solid lubricant receptivity (Area occupancy) |           |           |           |                                       |                  |
|-----------------------|----------------------------------------------|-----------|-----------|-----------|---------------------------------------|------------------|
|                       | WRa (LLH)                                    | WRa (LMH) | WRa (LHH) | WRa (LML) | (%) of zinc stearate on photoreceptor | Image evaluation |
| Example 1             | 0.039                                        | 0.008     | 0.015     | 0.012     | 14.0                                  | 5                |
| Example 2             | 0.027                                        | 0.010     | 0.016     | 0.010     | 12.8                                  | 5                |
| Example 3             | 0.027                                        | 0.016     | 0.017     | 0.015     | 10.9                                  | 5                |
| Example 4             | 0.024                                        | 0.011     | 0.017     | 0.012     | 15.2                                  | 5                |
| Example 5             | 0.031                                        | 0.015     | 0.018     | 0.013     | 12.2                                  | 5                |
| Example 6             | 0.028                                        | 0.012     | 0.016     | 0.013     | 10.1                                  | 5                |
| Example 7             | 0.019                                        | 0.011     | 0.015     | 0.013     | 12.7                                  | 5                |
| Comparative Example 1 | 0.019                                        | 0.003     | 0.002     | 0.004     | 1.9                                   | 2                |
| Comparative Example 2 | 0.018                                        | 0.002     | 0.002     | 0.005     | 1.6                                   | 3                |
| Comparative Example 3 | 0.021                                        | 0.002     | 0.001     | 0.004     | 0.6                                   | 1                |
| Comparative Example 4 | 0.025                                        | 0.004     | 0.002     | 0.007     | 3.0                                   | 1                |
| Comparative Example 5 | 0.048                                        | 0.030     | 0.003     | 0.050     | 3.4                                   | 3                |
| Comparative Example 6 | 0.026                                        | 0.002     | 0.009     | 0.025     | 6.0                                   | 3                |
| Comparative Example 7 | 0.031                                        | 0.022     | 0.038     | 0.018     | 6.5                                   | 3                |

The photoreceptors of Examples 1 to 7 satisfy the inequations (i) to (v). They have better solid lubricant receptivity than the photoreceptor of Comparative Example 1, the surface of which is not roughened. However, it is clear from the results of Comparative Example 3 that roughening of the surface not always improves solid lubricant receptivity.

When the surface of a photoreceptor has a surface with an appropriate roughness, i.e., the inequations (i) to (v) are satisfied, a solid lubricant does not sideslip on the photoreceptor

and an application blade causes appropriate variation in linear pressure, both of which may result in improvement of solid lubricant receptivity. The former is achieved by a high-frequency surface roughness and the latter is achieved by a low-frequency surface roughness.

Such a surface with an appropriate roughness can be obtained by adding a cross-linkable silicone material and a non-cross-linkable silicone material to a cross-linked resin surface layer coating liquid.

## Example 8

On each of an aluminum cylinder having a thickness of 0.8 mm, a length of 340 mm, and an outer diameter of 40 mm, and another aluminum cylinder having a thickness of 0.8 mm, a length of 340 mm, and an outer diameter of 30 mm, a undercoat layer coating liquid, a charge generation layer coating liquid, and a charge transport layer coating liquid are sequentially coated and dried in this order. Thus, an undercoat layer, a charge generation layer, and a charge transport layer having a thickness of 3.5  $\mu$ m, 0.2  $\mu$ m, and 24  $\mu$ m, respectively, are formed on each of the aluminum cylinders.

Further, a thermoplastic resin surface layer coating liquid is spray-coated on the aluminum cylinders having the undercoat layer, the charge generation layer, and the charge transport layer thereon, followed by drying for 10 minutes. The aluminum cylinders are put 120 mm away from a UV curing lamp so that the thermoplastic resin surface layer coating liquid is

subjected to UV curing while rotating. The illuminance at that position is 550 mW/cm<sup>2</sup> when measured with an accumulated UV meter UIT-150 from Ushio Inc. The aluminum cylinders rotate at a revolution of 25 rpm. The aluminum cylinders are exposed to UV ray for 4 minutes while circulating water having a temperature of 30° C. therein, followed by drying for 30 minutes at 130° C. Thus, photoreceptors having a thermoplastic resin surface layer having a thickness of 6  $\mu$ m are prepared.

53

The compositions of the coating layers are shown in Tables 10 to 13.

TABLE 10

| Composition of Undercoat Layer Coating Liquid |                                                 |                |
|-----------------------------------------------|-------------------------------------------------|----------------|
| Components                                    | Trade Name or Chemical Formula                  | Amount (parts) |
| Alkyd resin solution                          | BECKOLITE M6401-50 (from DIC Corporation)       | 12             |
| Melamine resin solution                       | SUPER BECKAMINE G-821-60 (from DIC Corporation) | 8.0            |

54

TABLE 10-continued

| Composition of Undercoat Layer Coating Liquid |                                           |                |
|-----------------------------------------------|-------------------------------------------|----------------|
| Components                                    | Trade Name or Chemical Formula            | Amount (parts) |
| Titanium oxide                                | CR-EL (from Ishihara Sangyo Kaisha, Ltd.) | 40             |
| Methyl ethyl ketone                           | —                                         | 200            |

TABLE 11

| Composition of Charge Generation Layer Coating Liquid |                                |                |
|-------------------------------------------------------|--------------------------------|----------------|
| Components                                            | Trade Name or Chemical Formula | Amount (parts) |
| Bisazo pigment                                        | <br>(from Ricoh Co., Ltd.)     | 5.0            |
| Polyvinyl butyral                                     | XYHL (from UCC)                | 1              |
| Cyclohexanone                                         | —                              | 200            |
| Methyl ethyl ketone                                   | —                              | 80             |

TABLE 12

| Composition of Charge Transport Layer Coating Liquid |                                                |                |
|------------------------------------------------------|------------------------------------------------|----------------|
| Components                                           | Trade Name or Chemical Formula                 | Amount (parts) |
| Z-type Polycarbonate                                 | PANLITE ® TS-2050 (from Teijin Chemicals Ltd.) | 10             |
| Low-molecular-weight charge transport material       |                                                | 7.0            |
| Tetrahydrofuran                                      | —                                              | 100            |
| Silicone oil (in 1% THF solution)                    | KF50-100CS (from Shin-Etsu Chemical Co., Ltd.) | 1              |

TABLE 13

| Composition of Thermoplastic Resin Surface Layer Coating Liquid |                                                 |                   |
|-----------------------------------------------------------------|-------------------------------------------------|-------------------|
| Components                                                      | Trade Name or Chemical Formula                  | Amount<br>(parts) |
| Z-type Polycarbonate                                            | PANLITE ® TS-2050 (from Teijin Chemicals Ltd.)  | 10                |
| Low-molecular-weight charge transport material                  |                                                 | 10.0              |
| Tetrahydrofuran                                                 | —                                               | 300               |
| Cyclohexanone                                                   | —                                               | 100               |
| Cross-linkable silicone oil material                            | X-22-174DX (from Shin-Etsu Chemical Co., Ltd.)  | 0.45              |
| Non-cross-linkable silicone oil material                        | KF-50-100CS (from Shin-Etsu Chemical Co., Ltd.) | 0.15              |

## Example 9

30

The procedure in Example 8 is repeated except for changing the amount of the cross-linkable silicone oil material to 0.75 parts.

## Example 10

35

The procedure in Example 8 is repeated except for changing the amount of the non-cross-linkable silicone oil material to 0.45 parts.

## Example 11

40

The procedure in Example 8 is repeated except for changing the amounts of the cross-linkable silicone oil material and the non-cross-linkable silicone oil material to 0.75 parts and 0.45 parts, respectively.

## Example 12

45

The procedure in Example 8 is repeated except for changing the amounts of the cross-linkable silicone oil material and the non-cross-linkable silicone oil material to 0.15 parts and 0.75 parts, respectively.

## Example 13

30

The procedure in Example 8 is repeated except for changing the amounts of the cross-linkable silicone oil material and the non-cross-linkable silicone oil material to 0.45 parts and 0.75 parts, respectively.

## Example 14

40

The procedure in Example 8 is repeated except for changing the amounts of the cross-linkable silicone oil material and the non-cross-linkable silicone oil material to 0.75 parts and 0.75 parts, respectively.

## Comparative Example 8

45

The procedure in Example 8 is repeated except for replacing the thermoplastic resin surface layer coating liquid with another thermoplastic resin surface layer coating liquid having the composition shown in Table 14.

TABLE 14

| Composition of Thermoplastic Resin Surface Layer Coating Liquid |                                                |                   |
|-----------------------------------------------------------------|------------------------------------------------|-------------------|
| Components                                                      | Trade Name or Chemical Formula                 | Amount<br>(parts) |
| Z-type Polycarbonate                                            | PANLITE ® TS-2050 (from Teijin Chemicals Ltd.) | 10                |

TABLE 14-continued

| Composition of Thermoplastic Resin Surface Layer Coating Liquid |                                |                |
|-----------------------------------------------------------------|--------------------------------|----------------|
| Components                                                      | Trade Name or Chemical Formula | Amount (parts) |
| Low-molecular-weight charge transport material                  |                                | 10.0           |
| Tetrahydrofuran                                                 | —                              | 300            |
| Cyclohexanone                                                   | —                              | 100            |

### Comparative Example 9

The procedure in Example 8 is repeated except for replacing the thermoplastic resin surface layer coating liquid with another thermoplastic resin surface layer coating liquid having the composition shown in Table 15.

TABLE 15

Composition of Thermoplastic Resin Surface Layer Coating Liquid

| Components                                     | Trade Name or Chemical Formula                                                      | Amount<br>(parts) |
|------------------------------------------------|-------------------------------------------------------------------------------------|-------------------|
| Z-type Polycarbonate                           | PANLITE ® TS-2050 (from Teijin Chemicals Ltd.)                                      | 10                |
| Low-molecular-weight charge transport material |  | 10.0              |
| Tetrahydrofuran                                | —                                                                                   | 300               |
| Cyclohexanone                                  | —                                                                                   | 100               |
| Non-cross-linkable silicone oil material       | KF-50-100CS (from Shin-Etsu Chemical Co., Ltd.)                                     | 0.15              |

### Comparative Example 10

The procedure in Example 8 is repeated except for replacing the thermoplastic resin surface layer coating liquid with another thermoplastic resin surface layer coating liquid having the composition shown in Table 16. 65

TABLE 16

| Composition of Thermoplastic Resin Surface Layer Coating Liquid |                                                                                   |                   |
|-----------------------------------------------------------------|-----------------------------------------------------------------------------------|-------------------|
| Components                                                      | Trade Name or Chemical Formula                                                    | Amount<br>(parts) |
| Z-type Polycarbonate                                            | PANLITE ® TS-2050 (from Teijin Chemicals Ltd.)                                    | 10                |
| Low-molecular-weight charge transport material                  |  | 10.0              |
| Tetrahydrofuran                                                 | —                                                                                 | 300               |
| Cyclohexanone                                                   | —                                                                                 | 100               |
| Cross-linkable silicone oil material                            | X-22-174DX (from Shin-Etsu Chemical Co., Ltd.)                                    | 0.45              |

Each of the photoreceptors prepared in Examples 8 to 14 and Comparative Examples 8 to 10 each having a diameter of 40 mm is mounted on a yellow development station of an image forming apparatus IPSIO SP C811 (from Ricoh Co., Ltd.) to be subjected to the solid lubricant receptivity test in the same manner as Example 1.

Next, each of the photoreceptors prepared in Examples 8 to 14 and Comparative Examples 8 to 10 each having a diameter of 40 mm is mounted on a black development station of an image forming apparatus IPSIO SP C811 (from Ricoh Co., Ltd.) to be subjected to the image evaluation in the same manner as Example 1.

The measurement results of WRa in Examples 8 to 14 and Comparative Examples 8 to 10 are shown in FIGS. 38 to 47. The results of WRa's, the solid lubricant receptivity test, and the image evaluation in Examples 8 to 14 and Comparative Examples 8 to 10 are shown in Table 17.

The photoreceptors of Examples 8 to 14 satisfy the inequations (i) to (v). They have better solid lubricant receptivity than the photoreceptor of Comparative Example 8, the surface of which is not roughened. However, it is clear from the results of Comparative Examples 9 and 10 that roughening of the surface not always improves solid lubricant receptivity.

When the surface of a photoreceptor has a surface with an appropriate roughness, i.e., the inequations (i) to (v) are satisfied, a solid lubricant does not sideslip on the photoreceptor and an application blade causes appropriate variation in linear pressure, both of which may result in improvement of solid lubricant receptivity. The former is achieved by a high-frequency surface roughness and the latter is achieved by a low-frequency surface roughness.

TABLE 17

|                           | Solid lubricant<br>receptivity<br>(Area occupancy<br>(%) of zinc stearate<br>on photoreceptor) |              |              |              |              |                     |
|---------------------------|------------------------------------------------------------------------------------------------|--------------|--------------|--------------|--------------|---------------------|
|                           | WRa<br>(LLH)                                                                                   | WRa<br>(LMH) | WRa<br>(LHH) | WRa<br>(LML) | WRa<br>(LML) | Image<br>evaluation |
| Example 8                 | 0.050                                                                                          | 0.008        | 0.015        | 0.012        | 13.0         | 5                   |
| Example 9                 | 0.049                                                                                          | 0.010        | 0.016        | 0.010        | 13.1         | 5                   |
| Example 10                | 0.048                                                                                          | 0.016        | 0.017        | 0.015        | 12.2         | 5                   |
| Example 11                | 0.051                                                                                          | 0.011        | 0.017        | 0.012        | 15.0         | 5                   |
| Example 12                | 0.052                                                                                          | 0.015        | 0.018        | 0.013        | 11.1         | 5                   |
| Example 13                | 0.050                                                                                          | 0.012        | 0.016        | 0.013        | 12.1         | 5                   |
| Example 14                | 0.048                                                                                          | 0.011        | 0.015        | 0.013        | 11.1         | 5                   |
| Comparative<br>Example 8  | 0.051                                                                                          | 0.030        | 0.003        | 0.050        | 1.0          | 1                   |
| Comparative<br>Example 9  | 0.052                                                                                          | 0.002        | 0.009        | 0.025        | 1.5          | 1                   |
| Comparative<br>Example 10 | 0.048                                                                                          | 0.022        | 0.038        | 0.018        | 3.5          | 2                   |

## 61

Such a surface with an appropriate roughness can be obtained by adding a cross-linkable silicone material and a non-cross-linkable silicone material to a thermoplastic resin surface layer coating liquid.

Additional modifications and variations of the present invention are possible in light of the above teachings. It is therefore to be understood that within the scope of the appended claims the invention may be practiced other than as specifically described herein.

## 62

( $\mu\text{m}$ ) of 26 to 106, 53 to 183, 106 to 318, 214 to 551, 431 to 954, and 867 to 1,654, respectively.

2. The electrophotographic photoreceptor according to claim 1, wherein the cross-linked resin surface layer comprises a cross-linked body of a cross-linkable charge transport material having a triarylamine structure.

3. The electrophotographic photoreceptor according to claim 1, wherein the cross-linked resin surface layer comprises a cross-linked body of a cross-linkable charge transport material having the following formula (A) in an amount of 5% by weight or more and 60% by weight or less:



What is claimed is:

1. An electrophotographic photoreceptor, comprising:  
a conductive substrate;  
a photosensitive layer located overlying the conductive substrate; and  
a surface layer located overlying the photosensitive layer, wherein  
the surface layer is a cross-linked resin surface layer formed by coating and curing a cross-linked resin surface layer coating liquid on the photosensitive layer, and  
the cross-linked resin surface layer coating liquid comprises a cross-linkable charge transport material, a trimethylolpropane triacrylate, a cross-linkable silicone material, and a non-cross-linkable silicone material,  
wherein the following inequations are satisfied:

$$0.005 < WRa(LMH) < 0.03 \quad (i)$$

$$0.010 < WRa(LHH) < 0.03 \quad (ii)$$

$$0.005 < WRa(LML) < 0.20 \quad (iii)$$

$$WRa(LLH) > WRa(LMH) \quad (iv)$$

$$WRa(LLH) > WRa(LHH) \quad (v)$$

wherein WRa ( $\mu\text{m}$ ) represents a center-line average roughness of frequency components LHH, LHL, LMH, LML, LLH, and LLL that are obtained by a method comprising:

subjecting a one-dimensional data array of a surface profile of the electrophotographic photoreceptor, which is measured with a surface roughness & profile shape measuring instrument, to wavelet transformation multiresolution analysis so as to be separated into 6 frequency components each having a cycle length ( $\mu\text{m}$ ) of 0 to 3, 1 to 6, 2 to 13, 4 to 25, 10 to 50, and 24 to 99;

thinning a one-dimensional data array of the lowest frequency component having a cycle length of from 24 to 99 ( $\mu\text{m}$ ) so that the number of data array is reduced to  $\frac{1}{40}$ ; and

subjecting the thinned one-dimensional data array to wavelet transformation multiresolution analysis so as to be separated into the 6 frequency components LHH, LHL, LMH, LML, LLH, and LLL each having a cycle length

25 where each of d, e, and f independently represents an integer of 0 or 1; each of g and h independently represents an integer of from 0 to 3; R<sub>13</sub> represents a hydrogen atom or a methyl group; each of R<sub>14</sub> and R<sub>15</sub> independently represents an alkyl group having 1 to 6 carbon atoms, wherein multiple R<sub>14</sub> and R<sub>15</sub> may be, but need not necessarily be, the same; and Z represents a single bond, a methylene group, an ethylene group,  $-\text{CH}_2\text{CH}_2\text{O}-$ ,



35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9

**63**

9. An image forming apparatus, comprising:  
the electrophotographic photoreceptor according to claim  
1 configured to bear an electrostatic latent image;  
a brush roller configured to apply a solid lubricant to a  
surface of the electrophotographic photoreceptor;  
a blade configured to extend the solid lubricant on the  
surface of the electrophotographic photoreceptor; and  
a developing device configured to develop the electrostatic  
latent image with a toner to form a toner image.
10. The image forming apparatus according to claim 9, 10  
wherein the toner is a polymerization toner.
11. The image forming apparatus according to claim 9,  
wherein the developing device is a tandem developing device

**64**

which includes 2 or more developing stations each configured  
to form different-color toner images with different-color  
polymerization toners.

12. A process cartridge detachably mountable on image  
5 forming apparatus, comprising:  
the electrophotographic photoreceptor according to claim  
1 configured to bear an electrostatic latent image;  
a brush roller configured to apply a solid lubricant to a  
surface of the electrophotographic photoreceptor; and  
a blade configured to extend the solid lubricant on the  
surface of the electrophotographic photoreceptor.

\* \* \* \* \*

UNITED STATES PATENT AND TRADEMARK OFFICE  
**CERTIFICATE OF CORRECTION**

PATENT NO. : 8,293,439 B2  
APPLICATION NO. : 12/723058  
DATED : October 23, 2012  
INVENTOR(S) : Yukio Fujiwara et al.

Page 1 of 1

It is certified that error appears in the above-identified patent and that said Letters Patent is hereby corrected as shown below:

Replace Item (54), Title, on the Title Page of the patent and Column 1, lines 1-6 in the specifications with the following:

-- ELECTROPHOTOGRAPHIC PHOTORECEPTOR, METHOD OF  
MANUFACTURING ELECTROPHOTOGRAPHIC  
PHOTORECEPTOR, IMAGE FORMING APPARATUS, AND  
PROCESS CARTRIDGE --

Signed and Sealed this  
Fifth Day of March, 2013



Teresa Stanek Rea  
*Acting Director of the United States Patent and Trademark Office*